



US006153352A

# United States Patent [19]

Oohashi et al.

[11] Patent Number: 6,153,352

[45] Date of Patent: Nov. 28, 2000

[54] **PLANOGRAPHIC PRINTING PLATE PRECURSOR AND A METHOD FOR PRODUCING A PLANOGRAPHIC PRINTING PLATE**

[75] Inventors: **Hidekazu Oohashi; Koichi Kawamura; Tadahiro Sorori; Morio Yagihara; Sumiaki Yamasaki**, all of Shizuoka-ken, Japan

[73] Assignee: **Fuji Photo Film Co., Ltd.**, Minami-Ashigara, Japan

[21] Appl. No.: **09/207,682**

[22] Filed: **Dec. 9, 1998**

[30] **Foreign Application Priority Data**

Dec. 10, 1997 [JP] Japan ..... 9-340358  
Dec. 24, 1997 [JP] Japan ..... 9-355798  
Feb. 26, 1998 [JP] Japan ..... 10-045635

[51] **Int. Cl. 7** ..... **G03C 1/76**

[52] **U.S. Cl.** ..... **430/270.1; 430/302**

[58] **Field of Search** ..... 430/270.1, 302, 430/271.1

[56] **References Cited**

U.S. PATENT DOCUMENTS

5,102,771 4/1992 Vogel et al. ..... 430/270  
5,340,693 8/1994 Uytterhoeven et al. ..... 430/253  
5,658,708 8/1997 Kondo ..... 430/288.1  
5,858,604 1/1999 Takeda et al. ..... 430/162  
5,948,591 9/1999 Vermeersch et al. ..... 430/270.1  
5,985,646 9/1999 Kawamura et al. ..... 430/192

FOREIGN PATENT DOCUMENTS

0 573 092 6/1992 European Pat. Off. .

0 559 248 9/1993 European Pat. Off. .  
0 652 483 5/1995 European Pat. Off. .  
0 703 499 3/1996 European Pat. Off. .  
0 855 267 7/1998 European Pat. Off. .  
0 869 394 10/1998 European Pat. Off. .

Primary Examiner—Janet Baxter  
Assistant Examiner—Barbara Gilmore  
Attorney, Agent, or Firm—Burns, Doane, Swecker & Mathis, LLP

[57] **ABSTRACT**

A planographic printing plate precursor which can be written by heat mode exposure of low energy, has excellent strength in image portions and blemishing resistance, can be developed with water, or can be installed in a printing machine as it is for conducting printing without requiring specific treatment such as wet developing treatment, rubbing and the like after writing of an image, and a method for producing the same, are provided. The planographic printing plate precursor of the present invention is obtained by laminating on a substrate having a hydrophilic surface a layer composed of a hydrophobic polymer which is made hydrophilic by heating and either a layer composed of a hydrophilic polymer compound having in the side chain at least one of alkylene oxide groups or functional groups selected from —COOR, —COOM, —SOR, —SO<sub>2</sub>R, —SO<sub>3</sub>R, —SOM, —SO<sub>2</sub>M, —SO<sub>3</sub>M, —OH, —NR<sup>22</sup>R<sup>23</sup> (wherein, R represent a hydrogen atom, alkyl group or aryl group, M represents a metal atom, R<sup>22</sup> and R<sup>23</sup> each independently represent a hydrogen atom, alkyl group or aryl group) or a layer of which exposed portions can be removed by heat mode exposure.

**5 Claims, No Drawings**

**PLANOGRAPHIC PRINTING PLATE  
PRECURSOR AND A METHOD FOR  
PRODUCING A PLANOGRAPHIC PRINTING  
PLATE**

**BACKGROUND OF THE INVENTION**

**1. Field of the Invention**

The present invention relates to a planographic printing plate precursor and a method for producing a planographic printing plate. More particularly, the present invention relates to a planographic printing plate precursor which can be produced by scanning exposure based on digital signals, and a simple method for producing a planographic printing plate using the same.

**2. Description of Related Art**

A conventional planographic printing plate has been produced by exposing a planographic printing plate precursor to a light through a lith film, then removing non-image portions by dissolving them in a developing solution. Recently, digitalizing technologies have been spread widely in which image information is electronically processed, stored, and output using a computer, and various new image output methods making use of such digitizing technologies have been put into actual use. As a result, a computer-to-plate technology in which active radioactive light having a high directivity such as a laser light is scanned according to image information in the form of digitized data and printing plate is directly produced not via a lith film is eagerly desired, and it is an important technological problem to obtain a printing plate precursor suitable for this. On the other hand, in conventional production processes for a planographic printing plate, a process wherein removing non-image portions by dissolving them after exposure is indispensable. However, since the developing waste solution thereof is alkaline, a method for producing a printing plate which does not require such a wet treatment is eagerly awaited in today's industrial world where great importance is attached to protecting the environment. Thus, because of the already developed technologies for digitalizing image information and the necessity of environmental protection, planographic printing plate precursors which do not require wet treatment and can be produced in dry mode are keenly sought.

Japanese Patent Application Laid-Open (JP-A) Nos. 5-77574, 4-125189, U.S. Pat. No. 5,187,047 and JP-A No. 62-195646 and the like disclose that after image formation, a film produced by sulfonation of polyolefins is used as a planographic printing plate precursor which does not require wet developing treatment, and hydrophilicity of the surface thereof is modified by thermal writing to create a plate precursor material which does not require developing treatment. In this system, an image is formed by de-sulfonating sulfone groups existing on the surface of photosensitive materials by thermal writing, therefore, developing treatment is not necessary, however, there is the drawback that noxious gas is generated in the writing.

U.S. Pat. Nos. 5,102,771 and 5,225,316 suggest a sensitive material obtained by combining a polymer having an acid-sensitive group in the side chain and a photo acid generator, and propose a non-developing system. This plate precursor has the drawbacks that the hydrophilicity thereof is low, it is easily contaminated, and the durability of the plate precursor and clearness of the printed image are inferior, since the acid generated is a carboxylic acid.

As image forming materials having radiation sensitivity suitable for the production of positive non-treated planographic printing plates, those described in JP-A No.

7-186562 are known using specific carboxylates or sulfonates as image forming materials. By using the image forming materials described in this publication, there can be obtained a planographic printing plate which can be developed with water giving a satisfactory print, however, if the energy in exposure is low, there is a tendency that the image forming material near the substrate does not become completely hydrophilic and the image forming material can not be removed completely, and accordingly, the resulting print is blemished.

Further, as a method for producing a printing plate by scanning exposure, a method has been suggested utilizing active radioactive light having a high power density. In general, the recording mode by high power density exposure is called heat mode recording. The reason for this is that in a high power density exposure system, it is believed that photo energy absorbed by a sensitive material is often converted into heat, and the desired phenomenon is caused by the heat generated. A large part of the merit in the heat mode recording method resides in the potential possibility of simple treatment, dry treatment, and no-treatment. This is based on the fact that the phenomenon utilized for image recording of a heat mode sensitive material does not substantially occur by exposure to a light of normal strength or under normal environmental temperatures thereby negating the necessity for image fixing after exposure.

As one preferable method of producing a planographic printing plate based on the heat mode recording, there is a method in which a hydrophobic image forming layer is provided on a hydrophilic substrate, the layer is subjected to image-wise heat mode exposure to alter the solubility and dispersibility of the hydrophobic layer, and where necessary, non-image portions are removed by wet development. As an example thereof, Japanese Patent Application Publication (JP-B) No. 46-27919 discloses a method in which a plate precursor comprising a hydrophilic substrate carrying thereon a recording layer which manifests improved solubility (a so-called positive), action by the effect of heat, and specifically a recording layer having a specific composition of saccharides, melamine-formaldehyde resin and the like, is subjected to heat mode recording to obtain a printing plate. However, heat mode scanning exposure sensitivity has been insufficient since none of the disclosed recording layers has satisfactory heat sensitivity. Further, it has been a practical problem that discrimination of hydrophobicity/hydrophilicity before and after exposure, namely a change in solubility is small. For example, for securing hydrophilicity after exposure, a recording layer is forced to become hydrophilic to a certain extent before exposure, and as a result, the ink receiving property of image portions of the resulting printing plate and strength in printing become insufficient.

On the other hand, as another heat mode positive type plate precursor, U.S. Pat. No. 3,574,657 and JP-A No. 50-113307 suggest a plate precursor having a constitution in which a hydrophobic recording layer which can be removed by heat mode exposure is provided on a hydrophilic substrate. The principle of image recording of this plate precursor is based on the fact that the layer structure of a recording layer is destroyed by exposure, and as a result, the recording layer is removed in the exposure or printing processes, unlike the above-described plate production based on a change in the solubility and dispersibility of a recording layer in a heat mode solution type positive plate precursor. However, in a heat mode exposure removal type positive plate precursor, complete removal of a hydrophobic recording layer is difficult, and manifestation of sufficient hydrophilicity of non-image portions is difficult. On the

other hand, there is the dilemma that when the thickness of a recording layer is decreased to enhance the removability thereof, a deterioration is caused in the strength of the image portions, and a printing plate having only a low printing resistance is obtained.

#### SUMMARY OF THE INVENTION

The present invention has been achieved in consideration of the above-described problems, and an object thereof is to provide a planographic printing plate precursor wherein after scanning exposure for a short period of time, exposed portions (non-image portions) have a high level of hydrophilicity and non-exposed portions (image portions) have a high level of hydrophobicity and strength. Namely, the object thereof is to provide a planographic printing plate precursor with which a planographic printing plate can be produced having excellent printing properties such as resistance to blemishes, printing durability and the like by scanning exposure for a short period of time. Another object thereof is to provide a planographic printing plate precursor with which a planographic printing plate can be produced also having excellent storage stability. Still another object thereof is to provide a method for producing a planographic printing plate which can be developed with water, or does not require additional wet treatment after exposure such as wet developing treatment, rubbing and the like after image writing.

The present inventors have studied intensively to solve the above-described problems, and as a result, found that an excellent planographic printing plate precursor for heat mode exposure is obtained by using a recording layer comprising a polymer compound having in the side chain a functional group which generates a hydrophilic group by heating, and an infrared absorbing agent. As a result of studies, it has been found that a plate precursor is obtained which can provide a planographic printing plate of which image portions have extremely excellent strength and resistance to blemishes, by providing on a substrate a heat sensitive layer composed of the above-described polymer which can be made hydrophilic by heating and a layer having specific functions, thereby achieving the present invention.

Namely, the planographic printing plate precursor of the present invention is obtained by laminating a layer composed of a hydrophobic polymer which can be made hydrophilic by heating (hereinafter, referred to as layer (b)) and either a layer composed of a hydrophilic polymer compound having at least one of alkylene oxide groups or having at least one functional groups selected from  $-\text{COOR}$ ,  $-\text{COOM}$ ,  $-\text{SOR}$ ,  $-\text{SO}_3\text{R}$ ,  $-\text{SOM}$ ,  $-\text{SO}_2\text{M}$ ,  $-\text{SO}_3\text{M}$ ,  $-\text{OH}$ ,  $-\text{NR}^{22}\text{R}^{23}$  (wherein, R represents a hydrogen atom, alkyl group, or aryl group, M represents a metal atom,  $\text{R}^{22}$  and  $\text{R}^{23}$  each independently represent a hydrogen atom, alkyl group, or aryl group) (hereinafter, referred to as a layer (a)) or a layer of which exposed portions can be removed by heat mode exposure (hereinafter, referred to as layer (c)).

In particular, the above-described problems are solved by (1) A planographic printing plate precursor obtained by laminating layer (a) and layer (b) in sequence on a substrate having a hydrophilic surface, (2) A planographic printing plate precursor obtained by laminating layer (b) and layer (c) in sequence on a substrate having a hydrophilic surface, or (3) A planographic printing plate precursor obtained by laminating layer (c) and layer (b) in sequence on a substrate having a hydrophilic surface.

In the above-described planographic printing plate precursor (1), when layer (b) composed of a hydrophobic polymer compound which has a specific functional group and is made hydrophilic by heating (hereinafter, referred to where appropriate as a heat sensitive polymer compound) is made hydrophilic image-wise by a specific heating means, because of the existence of a layer composed of a hydrophilic polymer compound which has a specific functional group (referred to as layer (a) including a layer containing only (a-1) described below, a layer containing only (a-2) described below and a layer containing one or more of these) between the substrate and layer (b), exposed portions of layer (b) can be made hydrophilic with high heat efficiency without scattering to the substrate of heat due to the exposure, as a result, sensitivity is improved, and in addition, layer (b) hydrophilized in non-image portions is solubilized with wetting water and does not remain on the substrate, therefore, the level of blemishing of the resulting print is extremely improved.

The above-described planographic printing plate precursor (2) of the present invention can provide a planographic printing plate which has very high sensitivity and is excellent in strength and blemish resistance of image portions by providing an intermediate layer having a specific function (layer (b)) below layer (c) in a planographic printing plate precursor comprising a substrate of which at least the surface is hydrophilic carrying thereon a lipophilic recording layer which can be removed by irradiation with active radioactive light having high energy density.

In the above-described planographic printing plate (3) light absorption and heat generation in heat mode exposure occur mainly in the intermediate layer (layer (c)) below heat sensitive layer (layer (b)), and the heat sensitive layer is made hydrophilic mainly from the substrate side. It is hypothesized that by this, hydrophilization of the heat sensitive layer becomes more complete. Further, the above-described planographic printing plate (3) manifests sufficient hydrophilicity even in the exposing energy range where hydrophilicity in non-image portions is insufficient on a conventional planographic printing plate precursor (a planographic printing plate precursor comprising a substrate carrying thereon only the intermediate layer of the present invention). Although the mechanism of this hydrophilicity manifestation is not clear, it is considered that providing a heat sensitive layer as an upper layer contributes to making the exposed portions hydrophilic. For example, it is considered that components in the intermediate layer and components in the heat sensitive layer may cause a certain chemical reaction and contribute to making the exposed portions hydrophilic.

#### DETAILED DESCRIPTION OF THE INVENTION

The above-described layer (a), layer (b) and layer (c) used in the planographic printing plate precursor of the present invention will be described below in detail.

##### Layer (a)

Layer (a) of the planographic printing plate precursor of the present invention is a layer mainly composed of a hydrophilic polymer compound (a-1) having in the side chain at least one functional group selected from  $-\text{COOR}$ ,  $-\text{COOM}$ ,  $-\text{SOR}$ ,  $-\text{SO}_3\text{R}$ ,  $-\text{SOM}$ ,  $-\text{SO}_2\text{M}$ ,  $-\text{SO}_3\text{M}$ ,  $-\text{OH}$ ,  $-\text{NR}^{22}\text{R}^{23}$  (wherein, R represents a hydrogen atom, alkyl group or aryl group, M represents a metal atom,  $\text{R}^{22}$  and  $\text{R}^{23}$  each independently represents a hydrogen atom, alkyl group or aryl group) or a hydrophilic polymer compound (a-2) having at least one alkylene oxide group.

The hydrophilicity of the hydrophilic polymer compound used in the present invention also includes the properties of water-solubility (meaning complete dissolving in water), pseudo water-solubility (meaning amphipatic properties, i.e. where the compound is water-soluble at a macroscopic level but contains non-soluble portions at a microscopic level), and water swelling (meaning the property where the compound swells with water but is not soluble in water). Namely, the compound contains a polymer which adsorbs or absorbs water under conditions of normal use or a polymer which is swollen with or dissolved in water. As compounds which lie within the above-described definition, a hydrophilic polymer compound (a-1) having at least one functional group selected from —COOR, —COOM, —SOR, —SO<sub>2</sub>R, —SO<sub>3</sub>R, —SOM, —SO<sub>2</sub>M, —SO<sub>3</sub>M, —OH, —NR<sup>22</sup>R<sup>23</sup> (wherein, R represents a hydrogen atom, alkyl group or aryl group, M represents a metal atom, R<sup>22</sup> and R<sup>23</sup> each independently represent a hydrogen atom, alkyl group, or aryl group) and a hydrophilic polymer compound (a-2) having in the molecule an alkylene oxide group are listed, and known natural polymer compounds or synthetic polymer compounds containing these functional groups can be used.

Examples of synthetic polymer compounds as the hydrophilic polymer compound (a-1) having at least one functional group selected from —COOR, —COOM, —SOR, —SO<sub>2</sub>R, —SO<sub>3</sub>R, —SOM, —SO<sub>2</sub>M, —SO<sub>3</sub>M, —OH, —NR<sup>22</sup>R<sup>23</sup> (wherein, R represents a hydrogen atom, alkyl group or aryl group, M represents a metal atom, R<sup>22</sup> and R<sup>23</sup> each independently represent a hydrogen atom, alkyl group or aryl group) include the following compounds: carboxylate salt-based copolymers, N-vinylcarboxylic amide-based copolymers, sulfonate salt-based copolymers, vinylpyrrolidone-based copolymers, polyvinyl alcohol, aqueous urethane resins, water-soluble polyesters, hydroxyethyl(meth)acrylate-based polymers, poly(vinylmethyl ether-co-maleic anhydride), polyethylene glycol di(meth)acrylate-based cross-linked polymers, polypropylene glycol di (meth)acrylate-based cross-linked polymers, and the like.

As the carboxylate salt-based copolymer having —COOR or —COOM in the side chain, there are listed saponification reaction products of carboxylic acid-based copolymers containing as a monomer component an  $\alpha,\beta$ -unsaturated compound having in the molecule one or two carboxyl groups or functional groups which can be converted to carboxyl groups such as a carboxyl group, carboxylate salt, carboxylic amide, carboxylic imide, carboxylic anhydride and the like.

Specific examples of the  $\alpha,\beta$ -unsaturated compound include acrylic acid, methacrylic acid, acrylates, methacrylates, acrylic amides, methacrylic amides, maleic anhydride, maleic acid, maleic amides, maleic imides, itaconic acid, crotonic acid, fumaric acid, mesaconic acid and the like.

Specific examples of the acrylates include methyl acrylate, ethyl acrylate, (n- or i-)propyl acrylate, (n-, i-, sec- or t-)butyl acrylate, amyl acrylate, 2-ethylhexyl acrylate, dodecyl acrylate, chloroethyl acrylate, 2-hydroxyethyl acrylate, 2-hydroxypropyl acrylate, 5-hydroxypentyl acrylate, cyclohexyl acrylate, allyl acrylate, trimethylolpropane monoacrylate, pentaerythritol monoacrylate, benzyl acrylate, methoxybenzyl acrylate, chlorobenzyl acrylate, hydroxybenzyl acrylate, hydroxyphenetyl acrylate, dihydroxyphenetyl acrylate, furfuryl acrylate, tetrahydrofurfuryl acrylate, phenyl acrylate, hydroxyphenyl acrylate, chlorophenyl acrylate, sulfamoylphenyl acrylate, 2-(hydroxyphenylcarbonyloxy)ethyl acrylate, and the like.

Specific examples of the methacrylates include methyl methacrylate, ethyl methacrylate, (n- or i-)propyl methacrylate, (n-, i-, sec- or t-)butyl methacrylate, amyl methacrylate, 2-ethylhexyl methacrylate, dodecylmethacrylate, chloroethyl methacrylate, 2-hydroxyethyl methacrylate, 2-hydroxypropyl methacrylate, 5-hydroxypentyl methacrylate, cyclohexyl methacrylate, allyl methacrylate, trimethylolpropane monomethacrylate, pentaerythritol monomethacrylate, glycidyl methacrylate, benzyl methacrylate, methoxybenzyl methacrylate, chlorobenzyl methacrylate, hydroxybenzyl methacrylate, hydroxyphenetyl methacrylate, dihydroxyphenetyl methacrylate, furfuryl methacrylate, tetrahydrofurfuryl methacrylate, phenyl methacrylate, hydroxyphenyl methacrylate, chlorophenyl methacrylate, sulfamoylphenyl methacrylate, 2-(hydroxyphenylcarbonyloxy)ethyl methacrylate, and the like.

Specific examples of the acrylamides include acrylamide, N-methylacrylamide, N-ethylacrylamide, N-propylacrylamide, N-butylacrylamide, N-benzylacrylamide, N-hydroxyethylacrylamide, N-phenylacrylamide, N-tolylacrylamide, N-(hydroxyphenyl)acrylamide, N-(sulfamoylphenyl)acrylamide, N-(phenylsulfonyl)acrylamide, N-(tolylsulfonyl)acrylamide, N,N-dimethylacrylamide, N-methyl-N-phenylacrylamide, N-hydroxyethyl-N-methylacrylamide, and the like.

Specific examples of the maleic amides include maleic amide, N-methylmaleic amide, N-ethylmaleic amide, N-propylmaleic amide, N-butylmaleic amide, N-benzylmaleic amide, N-hydroxyethylmaleic amide, N-phenylmaleic amide, N-tolylmaleic amide, N-(hydroxyphenyl)maleic amide, N-(sulfamoylphenyl)maleic amide, N-(phenylsulfonyl)maleic amide, N-(tolylsulfonyl)maleic amide, N,N-dimethylmaleic amide, N-methyl-N-phenylmaleic amide, N-hydroxyethyl-N-methylmaleic amide, and the like.

Specific examples of the maleic imides include maleic imide, N-methylmaleic imide, N-ethylmaleic imide, N-propylmaleic imide, N-butylmaleic imide, N-benzylmaleic imide, N-hydroxyethylmaleic imide, N-phenylmaleic imide, N-tolylmaleic imide, N-(hydroxyphenyl)maleic imide, N-(sulfamoylphenyl)maleic imide, N-(phenylsulfonyl)maleic imide, N-(tolylsulfonyl)maleic imide, and the like.

The carboxylate salt-based copolymers used in the present invention may be a homopolymer of the above-described  $\alpha,\beta$ -unsaturated compound, or a copolymer with another copolymerizable monomer providing it has hydrophilicity necessary to the present invention. Examples of the other copolymerizable monomer include known monomers such as ethylene, propylene, isobutylene, 1-butylene, diisobutylene, methyl vinyl ether, acrylonitrile, vinyl esters, styrenes and the like.

Specific examples of the vinyl esters include vinyl acetate, vinyl butyrate, vinyl benzoate, and the like.

Specific examples of the styrenes include styrene, methylstyrene, dimethylstyrene, trimethylstyrene, ethylstyrene, propylstyrene, cyclohexylstyrene, chloromethylstyrene, trifluoromethylstyrene, ethoxymethylstyrene, acetoxyethylstyrene, methoxystyrene, dimethoxystyrene, chlorostyrene, dichlorostyrene, bromostyrene, iodostyrene, fluorostyrene, carboxystyrene, and the like.

When combined with another monomer, the content of an  $\alpha,\beta$ -unsaturated compound containing a carboxyl group or a group which can be converted into a carboxyl group is

usually 10 mol % or more, and preferably 40 mol % or more in the whole monomer components.

A polymer contained as the  $\alpha,\beta$ -unsaturated compound containing a carboxyl group or a group which can be converted to a carboxyl group can be produced using known methods (see, e.g., POLYMER CHEMISTRY, vol. 7, p. 142 (1950)). Namely, these carboxylate salt copolymers may be any of random polymers, block polymers, graft polymers and the like, however, random polymers, appropriately selected depending on the polymerization method, are preferable. For example, they are synthesized by radical polymerization using polymerization initiators such as peroxides such as di-t-butyl peroxide, benzoyl peroxide and the like, persulfate salts such as ammoniumpersulfate and the like, azo compounds such as azobisisobutyronitrile and the like, as well as other compounds. As the polymerization method, solution polymerization, emulsion polymerization, suspension polymerization and the like are adopted.

Examples of suitable solvents used in synthesizing these carboxylate salt-based copolymers include tetrahydrofuran, ethylene dichloride, cyclohexanone, methyl ethyl ketone, acetone, methanol, ethanol, ethylene glycol monomethyl ether, ethylene glycol monoethyl ether, 2-methoxyethyl acetate, diethylene glycol dimethyl ether, 1-methoxy-2-propanol, 1-methoxy- 2-propyl acetate, N,N-dimethylformamide, N,N-dimethylacetamide, toluene, ethyl acetate, methyl lactate, ethyl lactate, dimethylsulfoxide, water and the like. These solvents are used alone or in combinations of two or more.

The degree of polymerization of these carboxylate salt-based copolymers is not particularly restricted.

The polymers or copolymers as explained above are preferably saponified in the presence of an alkaline catalyst. As the solvent used in the saponification, water, alcohol and aqueous alcohol solution are preferable. As the catalyst used for the saponification reaction, known alkaline catalysts are used, and particularly, alkaline metal hydroxides such as sodium hydroxide, potassium hydroxide and the like are suitable. The saponification reaction is accomplished by dissolving or dispersing the above-described polymer or copolymer in the above-described solvent, adding to this an alkaline catalyst and stirring the mixture for 1 to 10 hours at 20 to 80°C.

In the saponification reaction product in the present invention, the salt type thereof can be varied at will according to known methods. As salt-forming substances usually used, there are listed sodium hydroxide, potassium hydroxide, ammonium hydroxide, monomethylamine, dimethylamine, trimethylamine, monoethylamine, diethylamine, triethylamine, monoisopropylamine, diisopropylamine, triisopropylamine, monoethanolamine, diethanolamine, triethanolamine, monoisopropanolamine, diisopropanolamine, triisopropanolamine, N,N-dimethylethanolamine, N,N-dimethylisopropanolamine, cyclohexylamine, benzylamine, aniline, pyridine and the like.

Further, polyvalent metal salts of alkaline earth metal salts such as magnesium, potassium and the like can also be added in the form of a mixed salt with the above-described salts.

Specific examples of the carboxylate salt-based copolymers include compounds such as saponification reaction products of acrylic acid polymers, methacrylic acid polymers or methyl acrylate polymers, saponification reaction products of methacrylic amide copolymers, saponification reaction products of acrylic acid/methacrylic acid copolymers, maleic acid/styrene copolymers or methyl acrylate/vinyl acetate copolymers, and the like.

The term N-vinylcarboxylic amide-based copolymer means a copolymer containing as an essential repeating unit N-vinylcarboxylic amide (hereinafter, abbreviated as NVA) represented by the following general formula (6) (hereinafter, abbreviated as an NVA-based copolymer).

General formula (6)



wherein, R<sup>24</sup> represents a hydrogen atom or an alkyl group having 1 to 4 carbon atoms, R<sup>25</sup> represents a hydrogen atom, a methyl group, or phenyl group, and R<sup>26</sup> represents a hydrogen atom or a straight chain or branched chain alkyl group.

Specific examples of the NVA include, but are not limited to, N-vinylformamide, N-vinylpropionic amide, N-vinylbenzoic amide, N-methyl-N-vinylbenzoic amide, N-phenyl-N-vinylacetamide, N-phenyl-N-vinylbenzoic amide, and the like.

The N-vinylcarboxylic amide-based copolymer preferably used in the present invention preferably contains as a copolymer unit an  $\alpha,\beta$ -unsaturated compound having in the molecule one or two carboxyl groups or functional groups which can be derived into a carboxyl group such as a carboxyl group, carboxylate salt, carboxylic amide, carboxylic imide, carboxylic anhydride and the like.

Specific examples of the  $\alpha,\beta$ -unsaturated compound include acrylic acid, methacrylic acid, acrylates, methacrylates, acrylic amides, methacrylic amides, maleic anhydride, maleic acid, maleic amides, maleic imides, itaconic acid, crotonic acid, fumaric acid, mesaconic acid, and the like.

As the specific examples of the acrylates, methacrylates, acrylic amides, methacrylic amides, maleic amides and maleic imides, the compounds described above are listed.

The NVA-based copolymer preferably used in the present invention can contain another copolymerizable monomer providing it has the hydrophilicity necessary to the present invention. Examples of another copolymerizable monomer include known monomers such as ethylene, propylene, isobutylene, 1-butylene, diisobutylene, methyl vinyl ether, acrylonitrile, vinyl esters, styrenes and the like.

As specific examples of the vinyl esters and styrenes, the compounds described above are listed.

The NVA-based copolymer is usually prepared by radical polymerization. These NVA-based copolymers may be any polymer such as random polymers, block polymers, graft polymers and the like, and a random polymer which can be produced by known methods is preferable (see, e.g., POLYMER CHEMISTRY, vol. 7, p. 142 (1950)). Namely, these carboxylate salt-based copolymers may be any of random polymers, block polymers, graft polymers and the like, however, random polymers which are appropriately selected depending on the polymerization method are preferable. For example, they are synthesized by radical polymerization using polymerization initiators such as peroxides such as di-t-butyl peroxide, benzoyl peroxide and the like, persulfate salts such as ammonium persulfate and the like, azo compounds such as azobisisobutyronitrile and the like, as well as other compounds. As the polymerization method, solution polymerization, emulsion polymerization, suspension polymerization and the like are adopted.

Examples of suitable solvents used in synthesizing these NVA-based copolymers include tetrahydrofuran, ethylene dichloride, cyclohexanone, methyl ethyl ketone, acetone,

methanol, ethanol, ethylene glycol monomethyl ether, ethylene glycol monoethyl ether, 2-methoxyethyl acetate, diethylene glycol dimethyl ether, 1-methoxy-2-propanol, 1-methoxy-2-propyl acetate, N,N-dimethylformamide, N,N-dimethylacetamide, toluene, ethyl acetate, methyl lactate, ethyl lactate, dimethylsulfoxide, water and the like. These solvents are used alone or in combination of two or more.

The degree of polymerization of these NVA-based copolymers is not particularly restricted.

Specific examples of the NVA-based copolymer include the following polymers:

Poly(N-vinylacetamide), N-vinylacetamide/(meth) acrylic acid copolymer and partially or completely neutralized compound thereof (partially or completely neutralized compound means a copolymer in which a portion of all the hydrogen ions in a polymerizable functional group such as carboxylic acid, sulfonic acid, phosphoric acid and the like in the copolymer are substituted by an alkaline metal salt such as sodium, potassium and the like or an alkaline metal earth salt such as calcium, barium and the like), 15 N-vinylacetamide/crotonic acid copolymer and partially or completely neutralized compounds thereof, N-vinylacetamide/maleic acid copolymer and partially or completely neutralized compounds thereof, 20 N-vinylacetamide/fumaric acid copolymer and partially or completely neutralized compounds thereof, N-vinylacetamide/citraconic acid copolymer and partially or completely neutralized compounds thereof, 25 N-vinylacetamide/cinnamic acid copolymer and partially or completely neutralized compounds thereof, N-vinylacetamide/vinylsulfonic acid copolymer and partially or completely neutralized compounds thereof, N-vinylacetamide/maleic anhydride copolymer and partially or completely neutralized compounds thereof, 30 N-vinylacetamide/itaconic acid copolymer and partially or completely neutralized compounds thereof, N-vinylacetamide/aconic acid copolymer and partially or completely neutralized compounds thereof, 35 N-vinylacetamide/3-butenoic acid copolymer and partially or completely neutralized compounds thereof, N-vinylacetamide/4-pentenoic acid copolymer and partially or completely neutralized compounds thereof, 40 N-vinylacetamide/2-acryloyloxyethylphosphoric acid copolymer and partially or completely neutralized compounds thereof, N-vinylacetamide/3-acryloyloxypropylphosphoric acid copolymer and partially or completely neutralized compounds thereof, 45 N-vinylacetamide/methallylsulfonic acid copolymer and partially or completely neutralized compounds thereof, N-vinylacetamide/allylphosphoric acid copolymer and partially or completely neutralized compounds thereof, 50 N-vinylacetamide/carboxyethyl acrylate copolymer and partially or completely neutralized compounds thereof, N-vinylacetamide/2-acryloyloxyethylphosphoric acid copolymer and partially or completely neutralized compounds thereof, 55 N-vinylacetamide/2-acryloyloxypropylphosphoric acid copolymer and partially or completely neutralized compounds thereof, N-vinylacetamide/8-methacryloyloxyethylphosphoric acid copolymer and partially or completely neutralized compounds thereof, 60 N-vinylacetamide/2-acrylamide-n-propanesulfonic acid copolymer and partially or completely neutralized compounds thereof, N-vinylacetamide/2-acrylamide-n-octanesulfonic acid copolymer and partially or completely neutralized compounds thereof, N-vinylacetamide/2-acrylamide-2-methylpropanesulfonic acid copolymer and partially or completely neutralized compounds thereof, and the like.

As the sulfonate salt-based copolymer having in the side chain  $-\text{SO}_3\text{R}$  or  $-\text{SO}_3\text{M}$ , there are listed copolymers

containing as the monomer component an unsaturated compound having in the molecule a sulfonate salt or a functional group which can be derived into a sulfonate salt such as a sulfonic amide, sulfonate and the like, or saponification reaction products of the copolymers. As specific examples of such unsaturated compounds, the following compounds are listed.



Homopolymers obtained by using only one of these monomers may be used, however, copolymers obtained by using two or more of them and copolymers of these monomers with other monomers may also be used providing they manifest the hydrophilicity necessary to the present invention.

Examples of the copolymerizable other monomer include known monomers such as ethylene, propylene, isobutylene, 1-butylene, diisobutylene, methyl vinyl ether, acrylonitrile, acrylates, methacrylates, acrylamides, methacrylamides, vinyl esters, styrenes and the like.

Specific examples of the acrylates, methacrylates, acrylamides, methacrylamides, vinyl esters and styrenes include are as described above.

The polymer containing as a monomer an unsaturated compound containing a sulfonate salt or a group which can be converted to this is usually prepared by radical polymerization. These sulfonate salt-based copolymers may be any polymer such as random polymers, block polymers, graft polymers and the like, and a random polymer is preferable. They can be produced by known methods (see, e.g., POLYMER CHEMISTRY, vol. 7, p. 142 (1950)). Namely, these carboxylate salt copolymers may be any of random polymers, block polymers, graft polymers and the like, however, preferably, they are random polymers, and are appropriately selected depending on the polymerization method. For example, they are synthesized by radical polymerization using polymerization initiators such as peroxides such as di-t-butyl peroxide, benzoyl peroxide and the like, persulfate salts such as ammonium persulfate and the like, azo compounds such as azobisisobutyronitrile and the like, as well as other compounds. As the polymerization method, solution polymerization, emulsion polymerization, suspension polymerization and the like are adopted.

Examples of suitable solvents used in synthesizing these sulfonate salt-based copolymers include tetrahydrofuran, ethylene dichloride, cyclohexanone, methyl ethyl ketone,

## 11

acetone, methanol, ethanol, ethylene glycol monomethyl ether, ethylene glycol monoethyl ether, 2-methoxyethyl acetate, diethylene glycol dimethyl ether, 1-methoxy-2-propanol, 1-methoxy-2-propyl acetate, N,N-dimethylformamide, N,N-dimethylacetamide, toluene, ethyl acetate, methyl lactate, ethyl lactate, dimethylsulfoxide, water and the like. These solvents are used alone or in combinations of two or more.

The degree of polymerization of these sulfonate salt-based copolymers is not particularly restricted.

The copolymers as explained above are preferably saponified in the presence of an alkaline catalyst. As the solvent used in the saponification, water, alcohol and aqueous alcohol solution are preferable. As the catalyst used for the saponification reaction, known alkaline catalysts are used, and particularly, alkaline metal hydroxides such as sodium hydroxide, potassium hydroxide and the like are suitable. The saponification reaction is accomplished by dissolving or dispersing the above-described polymer or copolymer in the above-described solvent, adding to this an alkaline catalyst and stirring the mixture for 1 to 24 hours at 20 to 80° C.

In the saponification reaction product in the present invention, the type of salt can be varied at will according to known methods. As salt-forming substances usually used, there are listed sodium hydroxide, potassium hydroxide, ammonium hydroxide, monomethylamine, dimethylamine, trimethylamine, monoethylamine, diethylamine, triethylamine, monoisopropylamine, diisopropylamine, triisopropylamine, monoethanolamine, diethanolamine, triethanolamine, monoisopropanolamine, diisopropanolamine, triisopropanolamine, N,N-dimethylethanolamine, N,N-dimethylisopropanolamine, cyclohexylamine, benzylamine, aniline, pyridine and the like.

Further, polyvalent metal salts of alkaline earth metal salts such as magnesium, potassium and the like can also be added in the form of a mixed salt with the above-described salts.

Specific examples of the sulfonate salt-based copolymers include the following polymers:

(1)



(2)



(3)



## 12

-continued

(4)



(5)



Examples of polymers having preferable hydrophilicity for sufficiently manifesting the effect of the present invention in the above-described hydrophilic polymer compound include carboxylate salt-based copolymers, NVA-based copolymers, sulfonate salt-based copolymers and polyvinyl alcohol, and more preferably carboxylate salt-based copolymers, NVA-based copolymers and sulfonate salt-based copolymers.

Among the carboxylate salt-based copolymers, preferable are polymers or copolymers with acrylic acid and methacrylic acid, and copolymers of an a-olefin or vinyl compound with maleic anhydride, and more preferable are saponification reaction products of a vinyl ester with a (meth)acrylate copolymer (in the following explanation, (meth)acrylic acid is the abbreviation of acrylic acid and/or methacrylic acid). In this copolymer, it is preferable that the (meth)acrylate component occupies 20 to 80 mol % of the copolymer, and it is more preferable that the component occupies 30 to 70 mol % of the copolymer for satisfying simultaneously water absorption and mechanical strength requirements of the layer (a).

Among the NVA-based copolymers, preferable are copolymers of NVA with a carboxylic acid such as acrylic acid, methacrylic acid, maleic anhydride and the like, and from the viewpoints of water absorption and durability, the NVA unit occupies preferably 10 mol % or more, and more preferably 40 mol % or more of the whole monomer.

Further, preferable as the sulfonate salt-based copolymer are polymers and copolymers of styrenesulfonate salts and styrenesulfonates, copolymers of styrenesulfonate salts or styrenesulfonates with (meth)acrylic acid, (meth)acrylate, vinyl ester and/or maleic anhydride, or saponification reaction products of these polymers and copolymers. From the viewpoints of water absorption and durability, the styrenesulfonate salt or styrenesulfonate occupies preferably 20 mol % or more, and more preferably 50 mol % or more of the whole monomers.

Examples of natural polymer compounds as the hydrophilic polymer compounds having in the side chain a functional group selected from —COOR, —COOM, —SOR, —SO<sub>2</sub>R, —SO<sub>3</sub>R, —SOM, —SO<sub>2</sub>M, —SO<sub>3</sub>M, —OH, —NR<sup>22</sup>R<sup>23</sup> include starch-styrenesulfonic acid-based graft polymers, starch-vinylsulfonic acid-based graft polymers, starch-acrylamide-based graft polymers, carboxylated methylcellulose, cellulose-styrenesulfonic acid-based graft polymers, carboxymethylcellulose-based cross-linked compounds, and the like.

The hydrophilic polymer compound having an alkylene oxide group in the molecule (a-2) used in the present invention is not particularly restricted providing it has an alkylene oxide group in the main chain or side chain, specific examples thereof include polyethylene oxide, poly(ethylene oxide-co-propylene oxide) and the like, and examples of the natural polymer compound include starch-acrylonitrile-based graft polymer hydrolyzate, starch-acrylic acid-based graft polymers, methylcellulose,

## 13

hydroxypropylmethylcellulose, hydroxyethylcellulose, xanthic acid cellulose, cellulose-acrylonitrile-based graft copolymers, hyarulonic acid, agarose, collagen, milk casein, acid casein, rennet casein, ammonia casein, potassium casein, borax casein, glue, gelatin, gluten, soy bean protein, alginate, ammonium alginate, potassium alginate, sodium alginate, gum arabic, tragacanth gum, karaya gum, guar gum, locustbean gum, Irish moss, soy bean lecithin, pectinic acid, starch, carboxylated starch, agar, dextrin, mannan, and the like. The layer (a-1), (a-2) or (a) in the present invention may optionally contain compounds described below as constituent components in addition to the above-described hydrophilic polymer compounds within a range wherein the effect of the present invention is not lost.

Into the layer (a) of the planographic printing plate of the present invention, there can be added, for enhancing stability in the printing conditions, nonionic surfactants as described in JP-A Nos. 62-251740 and 3-208514, and ampholytic surfactants as described in JP-A Nos. 59-121044 and 4-13149.

Specific examples of the nonionic surfactant include sorbitan tristearate, sorbitan monopalmitate, sorbitantrioleate, stearic acid monoglyceride, polyoxyethylenenonyl phenyl ether, and the like.

Specific examples of the ampholytic surfactant include alkyldi(aminoethyl)glycine, alkylpolyaminoethylglycine hydrochloride, 2-alkyl-N-carboxyethyl-N-hydroxyethylimidazolinium betaine, N-tetradecyl-N,N-betaine type (for example, trade name: AMOGEN K, manufactured by Dai-itchi Kogyo Siyaku Co., Ltd.), and the like.

The proportion of the above-described nonionic surfactant and ampholytic surfactant based on the total weight of solid components of this hydrophilic layer is preferably from 0.05 to 15% by weight, and more preferably from 0.1 to 5% by weight.

A photo-thermal conversion material is preferably added to layer (a). Various infrared ray absorbing dyes can be preferably used as the photo-sensitive conversion material. The dye I represented by the following formula is especially preferable.



The layer (a) of the planographic printing plate of the present invention can be produced usually by dissolving the above-described components in a solvent and coating the mixture on a suitable substrate.

Examples of the solvent herein used include, but are not limited to, ethylene dichloride, cyclohexanone, methyl ethyl ketone, methanol, ethanol, propanol, ethylene glycol monomethyl ether, 1-methoxy-2-propanol, 2-methoxyethyl acetate, 1-methoxy-2-propyl acetate, dimethoxyethane, methyl lactate, ethyl lactate, N,N-dimethylacetamide, N,N-dimethylformamide, tetramethylurea, N-methylpyrrolidone,

## 14

dimethylsulfoxide, sulfolane, Y-butyrolactone, toluene, water, and the like.

These solvents are used alone or in a mixture. The concentration of the above-described components (whole solid components) in the solvent is preferably from 1 to 50% by weight.

Various methods can be used for the coating, and examples thereof include bar coater coating, rotation coating, spray coating, curtain coating, dip coating, air knife coating, blade coating, roll coating and the like.

Into the layer (a) of the planographic printing plate of the present invention, there can be added surfactants for enhancing coatability, for example, fluorine-based surfactants as described in JP-A No. 62-170950. The preferable amount added is from 0.01 to 1% by weight, and more preferably from 0.05 to 0.5% by weight based on the total weight of solid components in the layer (a).

Layer (a) manifests functions of securing a hydrophilic surface in exposed portions and improving heat efficiency, and therefore, the amount coated (solid component) on the substrate obtained after coating and drying is, in general, preferably from 0.5 mg/m<sup>2</sup> to 1.0 g/m<sup>2</sup>, more preferably from 1 mg/m<sup>2</sup> to 500 g/m<sup>2</sup>, and most preferably from 2 mg/m<sup>2</sup> to 300 g/m<sup>2</sup>.

When the amount coated is less than 0.5 g/m<sup>2</sup>, the effect for improving heat efficiency becomes insufficient, and even if the mixture is coated at an amount over 1.0 g/m<sup>2</sup>, improvement in the effect is not recognized, on the contrary, printing durability unpreferably deteriorates.

## Layer (b)

Layer (b) of the planographic printing plate precursor of the present invention changes to hydrophilic from hydrophobic and the solubility and dispersibility thereof the water increase by the action of heat. The change in hydrophobicity/hydrophilicity can be confirmed by for example solubility, dispersibility and wetting property (contact angle) in water. For example, a heat sensitive layer of which the contact angle against a water drop in air decreases by 10° or more by heating is preferable, and 40° or more is more preferable. Particularly preferably, the heat

sensitive layer is essentially insoluble in water before heating, and becomes soluble or dispersible in water by heating.

As preferable examples of the layer (b) having this property, there are listed polymers which can generate a sulfonic acid in the side chain by heating (hereinafter, referred to as "sulfonic acid generating polymers") and polymers which can generate a carboxylic acid in the side chain by heating (hereinafter, referred to as "carboxylic acid generating polymers"). These polymers, before heating, have a hydrophobic sulfonate or carboxylate structure and carry in the side chain a group which is converted to a

hydrophilic sulfonic acid structure or carboxylic acid structure by heating. Though carboxylates turn to carboxylic acids even by simply heating, it is preferable to use the carboxylates together with a compound which generates an acid by heating (hereinafter, referred to as "heat acid generator") since the reaction is accelerated in the presence of an acid. In addition, if the sulfonates are combined with a heat acid generator the reaction, may, in some cases, be accelerated.

The hydrophobic polymer compound is a polymer carrying in the side chain at least one of the groups represented by the above-described formulae (1) to (5). Sulfonic acid generating polymers having a group represented by the formulae (1) to (3) are preferable in that discrimination of hydrophobicity to hydrophilicity before and after recording by irradiation with a light is excellent.



Polymers which can generate a sulfonic acid in the side chain represented by the above-described formulae (1) to (3) by heating are described in detail below.

In the formulae (1) to (3), L represents an organic group composed of a polyvalent non-metal atom necessary for connecting a substituent to a polymer main chain. The substituent herein referred to is a sulfonate group.  $R^1$  represents a substituted or unsubstituted alkyl group, a substituted or unsubstituted aryl group, or a cyclic imide group,  $R^2$  and  $R^3$  represent a substituted or unsubstituted alkyl group or a substituted or unsubstituted aryl group,  $R^4$  represents a substituted or unsubstituted alkyl group, a substituted or unsubstituted aryl group, or  $-\text{SO}_2-\text{R}^5$ .  $R^5$  represents a substituted or unsubstituted alkyl group or a substituted or unsubstituted aryl group.

Preferable examples of  $R^1$  to  $R^5$  will be specifically described below. As the preferable example of the unsubstituted alkyl group  $R^1$ , straight chain, branched chain and cyclic alkyl groups having 1 to 20 carbon atoms are listed, and specific examples thereof include a methyl group, ethyl group, propyl group, butyl group, pentyl group, hexyl group, heptyl group, octyl group, nonyl group, decyl group, undecyl group, dodecyl group, tridecyl group, hexadecyl group, octadecyl group, eicosyl group, isopropyl group, isobutyl group, s-butyl group, t-butyl group, isopentyl group, neopentyl group, 1-methylbutyl group, isoheptyl group, 2-ethylhexyl group, 2-methylhexyl group, cyclohexyl group, cyclopentyl group, and 2-norbornyl group. Among these, straight-chain alkyl groups having 1 to 12 carbon atoms, branched-chain alkyl groups having 3 to 12 carbon atoms, and cyclic alkyl groups having 5 to 10 carbon atoms are preferable.

When  $R^1$  represents a substituted alkyl group, as the substituent of the substituted alkyl group, monovalent non-metal atom groups other than hydrogen are used, and preferable examples thereof include halogen atoms ( $-F$ ,  $-Br$ ,  $-Cl$ ,  $-I$ ), a hydroxyl group, alkoxy group, aryloxy group, mercapto group, alkylthio group, arylthio group, alkylidithio group, aryldithio group, amino group,  $N$ -alkylamino group,  $N,N$ -dialkylamino group,  $N$ -aryl amino

group, N,N-diaryl amino group, N-alkyl-N-aryl amino group, acyl amino group, carbamoyloxy group, N-alkylcarbamoyloxy group, N-arylcaramoyloxy group, N,N-dialkylcarbamoyloxy group, N,N-diarylcaramoyloxy group, N-alkyl-N-arylcaramoyloxy group, alkylsulfoxyl group, arylsulfoxyl group, acylthio group, acyl amino group, N-alkylacyl amino group, N-arylacyl amino group, ureido group, N'-alkylureido group, N',N'-dialkylureido group, N'-aryluureido group, N',N'-diaryluureido group, N'-alkyl-N'-aryluureido group, N-alkylureido group, N-aryluureido group, N-alkyl-N-alkylureido group, N-alkyl-N-aryluureido group, N',N'-dialkyl-N-aryluureido group, N'-aryl-N-aryluureido group, N'-aryl-N-alkylureido group, N-aryl-N-aryluureido group, N,N-diaryl-N-aryluureido group, N-alkyl-N'-aryl-N-aryluureido group, alkoxycarbonyl amino group, aryloxycarbonyl amino group, N-alkyl-N-alkoxycarbonyl amino group, N-alkyl-N-aryloxycarbonyl amino group, N-aryl-N-alkoxycarbonyl amino group, N-aryl-N-aryloxycarbonyl amino group, formyl group, acyl group, carboxyl group, alkoxycarbonyl group, aryloxycarbonyl group, carbamoyl group, N-alkylcarbamoyl group, N,N-dialkylcarbamoyl group, N-arylcaramoyl group, N,N-diarylcaramoyl group, N-alkyl-N-arylcaramoyl group, N-alkyl-N-arylcaramoyl group, N,N-dialkylsulfamoyl group, N-alkylsulfamoyl group, N,N-dialkylsulfamoyl group, N-arylsulfamoyl group, N,N-diarylsulfamoyl group, N-alkyl-N-arylsulfamoyl group, phosphono group ( $-\text{PO}_3\text{H}_2$ ) and conjugated basic groups thereof (hereinafter, abbreviated as a phosphonato group), dialkylphosphono group ( $-\text{PO}_3(\text{alkyl})_2$ ), diarylphosphono group ( $-\text{PO}_3(\text{aryl})_2$ ), alkylarylphosphono group ( $-\text{PO}_3(\text{alkyl})(\text{aryl})$ ), monoalkylphosphono group ( $-\text{PO}_3(\text{alkyl})$ ) monoarylphosphono group ( $-\text{PO}_3(\text{aryl})$ ) and conjugated basic groups thereof (hereinafter, abbreviated as an arylphosphonato group), phosphonoxy group ( $-\text{PO}_3\text{H}_2$ ) and conjugated basic groups thereof (hereinafter, abbreviated as a phosphonatoxy group), dialkylphosphonoxy group ( $-\text{OPO}_3(\text{alkyl})_2$ ), diarylphosphonoxy group ( $-\text{OPO}_3(\text{aryl})_2$ ), alkylarylphosphonoxy group ( $-\text{OPO}_3(\text{alkyl})(\text{aryl})$ ), monoalkylphosphonoxy group ( $-\text{OPO}_3\text{H}(\text{alkyl})$ ) and conjugated basic groups thereof (hereinafter, abbreviated as an alkylphosphonatoxy group), monoarylphosphonoxy group ( $-\text{OPO}_3\text{H}(\text{aryl})$ ) and conjugated basic group thereof (hereinafter, abbreviated as an arylphosphonatoxy group), cyano group, nitro group, aryl group, alkenyl group, and alkynyl group.

55 In the substituent of the substituted alkyl group, specific examples of the alkyl group include the alkyl groups as described above, and specific examples of the aryl group include a phenyl group, biphenyl group, naphthyl group, tolyl group, xyl group, mesityl group, cumenyl group, chlorophenyl group, bromophenyl group, chloromethylphenyl group, hydroxyphenyl group, methoxyphenyl group, ethoxyphenyl group, phenoxyphenyl group, acetoxyphenyl group, benzoxyloxyphenyl group, methylthiophenyl group, phenylthiophenyl group, methylaminophenyl group, dimethylaminophenyl group, acetylaminophenyl group, carboxyphenyl group, methoxycarbonylphenyl group, ethoxycarbonylphenyl group, phenoxy carbonylphenyl group, N-alkyl-N-alkylsulfamoyl group, N-alkyl-N-arylsulfamoyl group, N,N-dialkylsulfamoyl group, N-alkylsulfamoyl group, N,N-dialkylsulfamoyl group, N-arylsulfamoyl group, N,N-diarylsulfamoyl group, N-alkyl-N-arylsulfamoyl group, phosphono group ( $-\text{PO}_3\text{H}_2$ ) and conjugated basic groups thereof (hereinafter, abbreviated as a phosphonato group), dialkylphosphono group ( $-\text{PO}_3(\text{alkyl})_2$ ), diarylphosphono group ( $-\text{PO}_3(\text{aryl})_2$ ), alkylarylphosphono group ( $-\text{PO}_3(\text{alkyl})(\text{aryl})$ ), monoalkylphosphono group ( $-\text{PO}_3(\text{alkyl})$ ) monoarylphosphono group ( $-\text{PO}_3(\text{aryl})$ ) and conjugated basic groups thereof (hereinafter, abbreviated as an arylphosphonato group), phosphonoxy group ( $-\text{PO}_3\text{H}_2$ ) and conjugated basic groups thereof (hereinafter, abbreviated as a phosphonatoxy group), dialkylphosphonoxy group ( $-\text{OPO}_3(\text{alkyl})_2$ ), diarylphosphonoxy group ( $-\text{OPO}_3(\text{aryl})_2$ ), alkylarylphosphonoxy group ( $-\text{OPO}_3(\text{alkyl})(\text{aryl})$ ), monoalkylphosphonoxy group ( $-\text{OPO}_3\text{H}(\text{alkyl})$ ) and conjugated basic groups thereof (hereinafter, abbreviated as an alkylphosphonatoxy group), monoarylphosphonoxy group ( $-\text{OPO}_3\text{H}(\text{aryl})$ ) and conjugated basic group thereof (hereinafter, abbreviated as an arylphosphonatoxy group), cyano group, nitro group, aryl group, alkenyl group, and alkynyl group.

56 In the substituent of the substituted alkyl group, specific examples of the alkyl group include the alkyl groups as described above, and specific examples of the aryl group include a phenyl group, biphenyl group, naphthyl group, tolyl group, xyl group, mesityl group, cumenyl group, chlorophenyl group, bromophenyl group, chloromethylphenyl group, hydroxyphenyl group, methoxyphenyl group, ethoxyphenyl group, phenoxyphenyl group, acetoxyphenyl group, benzoxyloxyphenyl group, methylthiophenyl group, phenylthiophenyl group, methylaminophenyl group, dimethylaminophenyl group, acetylaminophenyl group, carboxyphenyl group, methoxycarbonylphenyl group, ethoxycarbonylphenyl group, phenoxy carbonylphenyl group, N-alkyl-N-alkylsulfamoyl group, N-alkyl-N-arylsulfamoyl group, N,N-dialkylsulfamoyl group, N-alkylsulfamoyl group, N,N-dialkylsulfamoyl group, N-arylsulfamoyl group, N,N-diarylsulfamoyl group, N-alkyl-N-arylsulfamoyl group, phosphono group ( $-\text{PO}_3\text{H}_2$ ) and conjugated basic groups thereof (hereinafter, abbreviated as a phosphonato group), dialkylphosphono group ( $-\text{PO}_3(\text{alkyl})_2$ ), diarylphosphono group ( $-\text{PO}_3(\text{aryl})_2$ ), alkylarylphosphono group ( $-\text{PO}_3(\text{alkyl})(\text{aryl})$ ), monoalkylphosphono group ( $-\text{PO}_3(\text{alkyl})$ ) monoarylphosphono group ( $-\text{PO}_3(\text{aryl})$ ) and conjugated basic groups thereof (hereinafter, abbreviated as an arylphosphonato group), phosphonoxy group ( $-\text{PO}_3\text{H}_2$ ) and conjugated basic groups thereof (hereinafter, abbreviated as a phosphonatoxy group), dialkylphosphonoxy group ( $-\text{OPO}_3(\text{alkyl})_2$ ), diarylphosphonoxy group ( $-\text{OPO}_3(\text{aryl})_2$ ), alkylarylphosphonoxy group ( $-\text{OPO}_3(\text{alkyl})(\text{aryl})$ ), monoalkylphosphonoxy group ( $-\text{OPO}_3\text{H}(\text{alkyl})$ ) and conjugated basic groups thereof (hereinafter, abbreviated as an alkylphosphonatoxy group), monoarylphosphonoxy group ( $-\text{OPO}_3\text{H}(\text{aryl})$ ) and conjugated basic group thereof (hereinafter, abbreviated as an arylphosphonatoxy group), cyano group, nitro group, aryl group, alkenyl group, and alkynyl group.

N-phenylcarbamoylphenyl group, phenyl group, cyanophenyl group, sulfophenyl group, sulfonatophenyl group, phosphonophenyl group, phosphonatophenyl group, and the like. Examples of an alkenyl group include a vinyl group, 1-propenyl group, 1-butenyl group, cinnamyl group, 2-chloro-1-ethenyl group, and the like. Examples of the alkenyl group include an ethynyl group, 1-propenyl group, 1-butynyl group, trimethylsilylethyynyl group, and the like. As  $G^1$  in the acyl group ( $G^1CO-$ ), hydrogen, and the above-described alkyl groups and aryl groups are listed. Among these substituents, more preferable examples include halogen atoms (—F, —Br, —Cl, —I), an alkoxy group, aryloxy group, alkylthio group, arylthio group, N-alkylamino group, N,N-dialkylamino group, acyloxy group, N-alkylcarbamoyloxy group, N-arylcaramoyloxy group, acylamino group, formyl group, acyl group, carboxyl group, alkoxy carbonyl group, aryloxy carbonyl group, carbamoyl group, N-alkylcarbamoyl group, N,N-dialkylcarbamoyl group, N-arylcaramoyl group, N-alkyl-N-arylcaramoyl group, sulfo group, sulfonato group, sulfamoyl group, N-alkylsulfamoyl group, N,N-dialkylsulfamoyl group, N-arylsulfamoyl group, N-alkyl-N-arylsulfamoyl group, phosphono group, phosphonato group, dialkylphosphono group, diarylphosphono group, monoalkylphosphono group, alkylphosphonato group, monoarylphosphono group, arylphosphonato group, phosphonoxy group, phosphonatoxy group, aryl group, and alkenyl group.

When  $R^1$  is a substituted alkyl group, as the alkylene group in the substituted alkyl group, there are listed divalent organic residual groups obtained by removing any one hydrogen atom from the above-described alkyl groups having 1 to 20 carbon atoms, and straight-chain alkylene groups having 1 to 12 carbon atoms, branched-chain alkylene groups having 3 to 12 carbon atoms and cyclic alkylene groups having 5 to 10 carbon atoms are preferable. Preferable specific examples of the substituted alkyl groups obtained by combining the above-described substituents with alkylene groups include a chloromethyl group, bromomethyl group, 2-chloroethyl group, trifluoromethyl group, methoxymethyl group, methoxyethoxyethyl group, allyloxymethyl group, phenoxyethyl group, methylthiomethyl group, tolylthiomethyl group, ethylaminethyl group, diethylaminopropyl group, morpholinopropyl group, acetylloxymethyl group, benzyloxymethyl group, N-cyclohexylcarbamoyloxyethyl group, N-phenylcarbamoyloxyethyl group, acetylaminoethyl group, N-methylbenzoylaminopropyl group, 2-oxoethyl group, 2-oxopropyl group, carboxypropyl group, methoxy-carbonylethyl group, allyloxycarbonylbutyl group, chlorophenoxy carbonylmethyl group, carbamoylmethyl group, N-methylcarbamoylethyl group, N,N-dipropylcarbamoylmethyl group, N-(methoxyphenyl) carbamoylethyl group, N-methyl-N-(sulfophenyl) carbamoylmethyl group, sulfobutyl group, sulfonatobutyl group, sulfamoylpropyl group, N-tolylsulfamoylpropyl group, N-methyl-N-(phosphonophenyl)sulfamoyloctyl group, phosphonobutyl group, phosphonatohexyl group, diethylphosphonobutyl group, diphenylphosphonopropyl group, methylphosphonobutyl group, methylphosphonato-butyl group, tolylphosphonohexyl group, tolylphosphonato-hexyl group, phosphonoxypropyl group, phosphonatoxybutyl group, benzyl group, phenyl group,  $\alpha$ -methylbenzyl group, 1-methyl-1-phenylethyl group, p-methylbenzyl group, cinnamyl group, allyl group, 1-propenylmethyl group, 2-butenyl group, 2-methylallyl group, 2-methylpropenylmethyl group, 2-propenylmethyl group, 2-butynyl group, 3-butynyl group, and the like.

When  $R^1$  is a unsubstituted aryl group, as preferable examples of the unsubstituted aryl group, condensed ring groups formed with 1 to 3 benzene rings, and condensed ring groups formed from a benzene ring and a 5-membered unsaturated ring, are listed, and specific examples thereof include a phenyl group, naphthyl group, anthryl group, phenanthryl group, indenyl group, acenaphthenyl group and fluorenyl group. Among these, a phenyl group and naphthyl group are more preferable. The aryl group includes, in addition to the above-described carbon cyclic aryl groups, heterocyclic aryl groups. As the heterocyclic aryl group, there are used those having 3 to 20 carbon atoms and 1 to 5 hetero atoms such as a pyridyl group, furyl group, and quinolyl group obtained by ring-condensation of a benzene group, benzofuryl group, thioxanthone group, carbazol groups and the like.

When  $R^1$  is a substituted aryl group, as examples of the substituted aryl group, the above-described type aryl groups carrying a monovalent non-metal atom group except hydrogen may be used as the substituent on ring-forming carbon atoms. As examples of preferable substituents, the above-described substituted or unsubstituted alkyl groups, and those previously exemplified as substituents on the substituted alkyl groups, are listed. Preferable specific examples of the substituted aryl group include a biphenyl group, tolyl group, xyl group, mesityl group, cumenyl group, chlorophenyl group, bromophenyl group, fluorophenyl group, chloromethylphenyl group, trifluoromethylphenyl group, hydroxyphenyl group, methoxyphenyl group, methoxyethoxyphenyl group, allyloxyphenyl group, phenoxyphenyl group, methylthiophenyl group, tolylthiophenyl group, ethylaminophenyl group, diethylaminophenyl group, morpholinophenyl group, acetoxyphenyl group, benzyloxyphenyl group, N-cyclohexylcarbamoyloxyphenyl group, N-phenylcarbamoyloxyphenyl group, acetylaminophenyl group, N-methylbenzoylaminophenyl group, carboxyphenyl group, methoxycarbonylphenyl group, allyloxycarbonylphenyl group, chlorophenoxy carbonylphenyl group, carbamoylphenyl group, N-methylcarbamoylphenyl group, N,N-dipropylcarbamoylphenyl group, N-(methoxyphenyl) carbamoylphenyl group, N-methyl-N-(sulfophenyl) carbamoylphenyl group, sulfophenyl group, sulfonatophenyl group, sulfamoylphenyl group, N-ethylsulfamoylphenyl group, N,N-dipropylsulfamoylphenyl group, N-tolylsulfamoylphenyl group, N-methyl-N-(phosphonophenyl)sulfamoylphenyl group, phosphonophenyl group, phosphonatophenyl group, diethylphosphonophenyl group, diphenylphosphonophenyl group, methylphosphonophenyl group, methylphosphonatophenyl group, tolylphosphonophenyl group, tolylphosphonatophenyl group, allyl group, 1-propenylmethyl group, 2-butenyl group, 2-methylallylphenyl group, 2-methylpropenylphenyl group, 2-propenylphenyl group, 2-butynylphenyl group, 3-butynylphenyl group and the like.

When  $R^1$  is a cyclic imide group, as preferable examples of the cyclic imide group, those having 4 to 20 carbon atoms such as succinic imide, phthalic imide, cyclohexanedicarboxylic imide, norbornenedicarboxylic imide and the like are listed.

Among other, it is particularly preferable from the view points of storability and heat decomposability when  $R^1$  is a primary or secondary alkyl which may have a substituent.

When  $R^2$  and  $R^3$  represent a substituted or unsubstituted alkyl group, or substituted or unsubstituted aryl group, preferable examples thereof are the same as the preferable examples of the substituted or unsubstituted alkyl group, or substituted or unsubstituted aryl group of  $R^1$ .

## 19

When  $R^4$  represents a substituted or unsubstituted alkyl group, or substituted or unsubstituted aryl group, preferable examples thereof are the same as the preferable examples of the substituted or unsubstituted alkyl group, or substituted or unsubstituted aryl group of  $R^1$ . When  $R^4$  is  $-\text{SO}_2-\text{R}^5$ ,  $R^5$  represents a substituted or unsubstituted alkyl group, or substituted or unsubstituted aryl group. When  $R^5$  represents a substituted or unsubstituted alkyl group, or substituted or unsubstituted aryl group, preferable examples thereof are the same as the preferable examples of the substituted or unsubstituted alkyl group, or substituted or unsubstituted aryl group of  $R^1$ .

$L$  connects a polymer main chain with a sulfonate group which is a substituent thereof, in a sulfonic acid generating polymer. The organic group composed of a polyvalent non-metal atom represented by  $L$  is an organic group composed of 1 to 60 carbon atoms, 0 to 10 nitrogen atoms, 0 to 50 oxygen atoms, 1 to 100 hydrogen atoms and 0 to 20 sulfur atoms. As more specific organic groups, those constituted of combinations of the following structural units are listed.



Polyvalent napthalene



Polyvalent anthracene



50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5240

5245

5250

5255

5260

5265

5270

5275

5280

5285

5290

5295

5300

5305

5310

5315

5320

5325

5330

5335

5340

5345

5350

5355

5360

5365

5370

5375

5380

5385

5390

5395

5400

5405

5410

5415

5420

5425

5430

5435

5440

5445

5450

5455

5460

5465

5470

5475

5480

5485

5490

5495

5500

5505

5510

5515

5520

5525

5530

5535

5540

5545

5550

5555

5560

5565

5570

5575

5580

5585

5590

5595

5600

5605

5610

5615

5620

5625

5630

5635

5640

5645

5650

5655

5660

5665

5670

5675

5680

5685

5690

5695

5700

5705

5710

5715

5720

5725

5730

5735

5740

5745

5750

5755

5760

5765

5770

5775

5780

5785

5790

5795

5800

5805

5810

5815

5820

5825

5830

5835

5840

5845

5850

5855

5860

5865

5870

5875

5880

5885

5890

5895

5900

5905

5910

5915

5920

5925

5930

5935

59

-continued



-continued

(1m-11)



5

(1m-7)

10

20

(1m-8)

30

35

(1m-9)

45

(1m-10)

55

60

65

(1m-12)

(1m-13)

(1m-14)

(1m-15)

(1m-16)



**23**

-continued



(1m-17)



(1m-18)



(1m-19)



(1m-20)



(1m-21)

5

10

15

20

25

30

35

40

45

50

55

60

**24**

-continued

(1m-22)



(1m-23)



(1m-24)



(1m-25)



(1m-26)



65

**25**

-continued



-continued



(1m-38)



(1m-39)



(1m-40)



For obtaining the sulfonic acid generating polymer, only one of the monomers having the partial structures represented by the formulae (1) to (3) described above may be homo-polymerized or two or more of the monomers may be copolymerized. Further, there may be used a copolymer obtained by copolymerizing a monomer having a partial structure represented by the formulae (1) to (3) with another monomer. As examples of such a copolymer, there are listed those obtained by radical-copolymerization of exemplified radical-polymerizable monomers with other radical-polymerizable monomers.

Examples of the other monomers used include known monomers such as acrylates, methacrylates, acrylamides, methacrylamides, vinyl esters, styrenes, acrylic acid, methacrylic acid, acrylonitrile, maleic anhydride, maleic imide and the like. By copolymerizing such monomers, various physical properties such as film formability, film strength, hydrophilicity, hydrophobicity, solubility, reactivity, stability and the like can be improved.

Specific examples of the acrylates include methyl acrylate, ethyl acrylate, (n- or i-)propyl acrylate, (n-, i-, sec- or t-)butyl acrylate, amyl acrylate, 2-ethylhexyl acrylate,

dodecyl acrylate, chloroethyl acrylate, 2-hydroxyethyl acrylate, 2-hydroxypropyl acrylate, 5-hydroxypentyl acrylate, cyclohexyl acrylate, allyl acrylate, trimethylolpropane monoacrylate, pentaerythritol monoacrylate, benzyl acrylate, methoxybenzyl acrylate, chlorobenzyl acrylate, hydroxybenzyl acrylate, hydroxyphenethyl acrylate, dihydroxyphenethyl acrylate, furfuryl acrylate, tetrahydrofurfuryl acrylate, phenyl acrylate, hydroxyphenyl acrylate, chlorophenyl acrylate, sulfamoylphenyl acrylate, 2-(hydroxyphenylcarbonyloxy)ethyl acrylate, and the like.

Specific examples of the methacrylates include methyl methacrylate, ethyl methacrylate, (n- or i-)propyl methacrylate, (n-, i-, sec- or t-)butyl methacrylate, amyl methacrylate, 2-ethylhexyl methacrylate, dodecyl methacrylate, chloroethyl methacrylate, 2-hydroxyethyl methacrylate, 2-hydroxypropyl methacrylate, 5-hydroxypentyl methacrylate, cyclohexyl methacrylate, allyl methacrylate, trimethylolpropane monomethacrylate, pentaerythritol monomethacrylate, glycidyl methacrylate, benzyl methacrylate, methoxybenzyl methacrylate, chlorobenzyl methacrylate, -hydroxybenzyl methacrylate, hydroxyphenethyl methacrylate, dihydroxyphenethyl methacrylate, furfuryl methacrylate, tetrahydrofurfuryl methacrylate, phenyl methacrylate, hydroxyphenyl methacrylate, chlorophenyl methacrylate, sulfamoylphenyl methacrylate, 2-(hydroxyphenylcarbonyloxy)ethyl methacrylate, and the like.

Specific examples of the acrylamides include acrylamide, N-methylacrylamide, N-ethylacrylamide, N-propylacrylamide, N-butylacrylamide, N-benzylacrylamide, N-hydroxyethylacrylamide, N-phenylacrylamide, N-tolylacrylamide, N-(hydroxyphenyl)acrylamide, N-(sulfamoylphenyl)acrylamide, N-(phenylsulfonyl)acrylamide, N,N-dimethylacrylamide, N-methyl-N-phenylacrylamide, N-hydroxyethyl-N-methylacrylamide, and the like.

Specific examples of the methacrylamides include methacrylamide, N-methylmethacrylamide, N-ethylmethacrylamide, N-propylmethacrylamide, N-butylmethacrylamide, N-benzylmethacrylamide, N-hydroxyethylmethacrylamide, N-phenylmethacrylamide, N-tolylmethacrylamide, N-(hydroxyphenyl)methacrylamide, N-(sulfamoylphenyl)methacrylamide, N-(phenylsulfonyl)methacrylamide, N-(tolylsulfonyl)methacrylamide, N,N-dimethylmethacrylamide, N-methyl-N-phenylmethacrylamide, N-hydroxyethyl-N-methylmethacrylamide, and the like.

Specific examples of the vinyl esters include vinyl acetate, vinyl butyrate, vinyl benzoate, and the like.

Specific examples of the styrenes include styrene, methylstyrene, dimethylstyrene, trimethylstyrene, ethylstyrene, propylstyrene, cyclohexylstyrene, chloromethylstyrene, trifluoromethylstyrene, ethoxymethylstyrene, acetoxyethylstyrene, methoxystyrene, dimethoxystyrene, chlorostyrene, dichlorostyrene, bromostyrene, iodostyrene, fluorostyrene, carboxystyrene, and the like.

As the other monomers, there may be used where necessary monomers having cross-linking reactivity such as glycidyl methacrylate, N-methylolmethacrylamide,  $\omega$ -(trimethoxysilyl)propyl methacrylate, 2-isocyanate ethyl acrylate and the like.

Among these other monomers, particularly suitably used are acrylates, methacrylates, acrylamides, methacrylamides, vinyl esters, styrenes, acrylic acid, methacrylic acid, and acrylonitrile having not more than 20 carbon atoms.

29

The proportion of these other monomers used for synthesizing a copolymer is required to be an amount sufficient for improving the various physical properties, however, when the proportion is too high, the function of the partial structure of the general formula (1) is insufficient. Therefore, the total proportion of preferable other monomers is preferably 80% by weight or less, and more preferably 50% by weight or less. 5

Specific examples of the sulfonic acid generating polymer in the present invention will be described below. <sup>10</sup>



31

-continued



-continued

(1p-15)



(1p-10)

5

(1p-11) 15

(1p-12) 25  
30

(1p-13) 40  
45

(1p-14)

**33**

-continued

**34**

-continued



-continued



(1p-28)

5



(1p-30)

(4)



(5)



The numbers in the formulae represent molar composition of the polymer compound.

Examples of solvents used in synthesizing the sulfonic acid generating polymer used in the present invention include tetrahydrofuran, ethylene dichloride, cyclohexanone, methyl ethyl ketone, acetone, methanol, ethanol, ethylene glycol monomethyl ether, ethylene glycol monoethyl ether, 2-methoxyethyl acetate, diethylene glycol dimethyl ether, 1-methoxy-2-propanol, 1-methoxy-2-propyl acetate, N,N-dimethylformamide, N,N-dimethylacetamide, toluene, ethyl acetate, methyl lactate, ethyl lactate, dimethylsulfoxide, water, and the like. These solvents are used alone or in combination of two or more.

As the polymerization initiator used in synthesizing the sulfonic acid generating polymer used in the present invention by radical polymerization, known compounds such as azo-based initiators, peroxide initiators and the like can be used.

The sulfonic acid generating polymer used in the present invention can be easily synthesized by methods known to those skilled in the art as described above. The polymerizable monomer is synthesized, for example, by de-hydrochlorination condensation of sulfonyl chloride with alcohol. Synthesis of the polymer can be carried out by the general procedure described above. A more specific synthesis method for the sulfonic acid generating polymer in the present invention is disclosed, for example, in Japanese Patent Application No. 9-026878.

Next, the polymer which generates a carboxylic acid in the side chain by heating, which is another example of the components of the layer (b) used in the present invention, will be described in detail below. As such a carboxylate polymer, for example, those described in JP-B No. 2-27660, JP-A Nos. 5-181279, 6-83059, 6-282073, European Patent Application No. 366590 and the like are listed.

As specific examples of the preferable carboxylic acid generating polymer, polymers are listed having in the side chain a group represented by the following general formulae (4) and (5).

In the formulae (4) and (5), L represents an organic group composed of a polyvalent non-metal atom necessary for connecting a substituent to a polymer main chain. The substituent herein referred to is a carboxylate. R<sup>6</sup> to R<sup>10</sup> may be the same or different, and represent a hydrogen atom, or an alkyl group, alkenyl group, acyl group or alkoxy carbonyl group which may have a substituent, and R<sup>11</sup> represents an alkyl group or alkenyl group which may have a substituent. Further, two of R<sup>6</sup> to R<sup>8</sup> or two of R<sup>9</sup> to R<sup>11</sup> may be connected to form a ring structure composed of 3 to 8 carbon atoms or hetero atoms.

Preferable examples of the alkyl group in which R<sup>6</sup> to R<sup>10</sup> may have a substituent include those having 1 to 8 carbon atoms which may have a substituent, such as a methyl group, ethyl group, propyl group, n-butyl group, sec-butyl group, hexyl group, 2-ethylhexyl group, and octyl group. Preferable examples when the alkyl group is a cycloalkyl group include those having 3 to 8 carbon atoms which may have a substituent, such as a cyclopropyl group, cyclopentyl group and cyclohexyl group. Preferable examples of the alkenyl group which may have a substituent include those having 2 to 6 carbon atoms which may have a substituent, such as a vinyl group, propenyl group, allyl group, butenyl group, pentenyl group, hexenyl group and cyclohexenyl group. Preferable examples of the acyl group which may have a substituent include those having 1 to 10 carbon atoms which may have a substituent, such as a formyl group, acetyl group, propanoyl group, butanoyl group, octanoyl group and the like. Preferable examples of the alkoxy carbonyl group which may have a substituent include those having 2 to 8 carbon atoms which may have a substituent, such as a methoxycarbonyl group, butoxycarbonyl group and the like.

Preferable examples when R<sup>11</sup> is an alkyl group and preferable examples when R<sup>11</sup> is an alkenyl group are the same as those for R<sup>6</sup> to R<sup>10</sup>.

When R<sup>6</sup> to R<sup>10</sup> and R<sup>11</sup> further have a substituent, preferable examples of the substituent include a hydroxyl group, halogen atoms (—F, —Cl, —Br, —I), a nitro group, cyano group, amide group, sulfonamide group, and further, alkoxy groups having 1 to 8 carbon atoms such as a methoxy group, ethoxy group, propoxy group, butoxy group and the like, and the alkyl groups, alkoxy carbonyl groups, acyl groups and cycloalkyl groups exemplified for R<sup>6</sup> to R<sup>10</sup>. When any two of R<sup>6</sup> to R<sup>10</sup> and R<sup>11</sup> on the same carbon atom are connected each other to form a ring, there are listed 3 to 8-membered rings which may have a hetero atom such as a cyclopropyl group, cyclopentyl group, cyclohexyl group, cycloheptyl group, tetrahydrofuran group, tetrahydropyran group and the like as the preferable ring. These may further have the above-described substituent.

L connects a polymer main chain with a carboxylate in a carboxylic acid generating polymer. Other conditions thereof are the same as those for L in the general formulae (1) to (3).

37

Among the polymers having a group represented by the general formulae (4) to (5), particularly preferable are polymers having at least one of the repeating units represented by the following formulae (7) to (12).



5

(7)



10

(8)



15

(9)



20

(10)

38

-continued

(11)



5

10

15

20

25

30



(12)

In the formulae (7) to (12), R<sup>12</sup> and R<sup>13</sup> may be the same or different and represent a hydrogen atom, cyano group, 35 alkyl group or haloalkyl group, R<sup>14</sup> represents a cyano group, —CO—OR<sup>15</sup> or —CONR<sup>16</sup>R<sup>17</sup>. R<sup>15</sup> to R<sup>17</sup> may be the same or different and represent a hydrogen atom, and an alkyl group, cycloalkyl group or alkenyl group which may have a substituent. R<sup>16</sup> and R<sup>17</sup> may be connected to each 40 other to form a ring. X<sup>0</sup> to X<sup>2</sup> may be the same or different, and represent a single bond, or an alkylene group, alkylene group or cycloalkylene group which may have a substituent, —O—, —SO<sub>2</sub>—, —O—CO—R<sup>18</sup>—, —CO—O—R<sup>19</sup>— or —CO—NR<sup>20</sup>—R<sup>21</sup>—. R<sup>18</sup>, R<sup>19</sup> and R<sup>21</sup> may 45 be the same or different, and represent a single bond, or a divalent alkylene group, alkenylene group or cycloalkylene group, and these groups may further form a divalent group together with an ether group, ester group, amide group, urethane group or ureide group. R<sup>20</sup> may represent a 50 hydrogen, or an alkyl group, cycloalkyl group or alkenyl group which may have a substituent. R<sup>6</sup> to R<sup>11</sup> have the same definitions as for the above-described general formulae (4) and (5).

As the alkyl groups R<sup>12</sup> and R<sup>13</sup>, there are listed those 55 having 1 to 4 carbon atoms which may have a substituent such as a methyl group, ethyl group, propyl group, n-butyl group and sec-butyl group. As the haloalkyl groups, there are preferably listed alkyl groups having 1 to 4 carbon atoms and substituted by a fluorine atom, chlorine atom or bromine 60 atom, for example, a fluoromethyl group, chloromethyl

group, bromomethyl group, fluoroethyl group, chloroethyl group, bromoethyl group and the like.

$R^{14}$  represents a cyano group,  $-\text{CO}-\text{OR}^{15}$  or  $-\text{CONR}^{16}\text{R}^{17}$ . As the alkyl groups  $\text{R}^{15}$  to  $\text{R}^{17}$ , there are listed those having 1 to 4 carbon atoms which may have a substituent, such as a methyl group, ethyl group, propyl group, n-butyl group and sec-butyl group. As the cycloalkyl group, there are preferably listed those having 3 to 8 carbon atoms which may have a substituent, such as a cyclopropyl group, cyclopentyl group and cyclohexyl group. As the alkenyl group, there are listed those having 2 to 6 carbon atoms which may have a substituent, such as a vinyl group, propenyl group, allyl group, butenyl group, pentenyl group, hexenyl group and cyclohexenyl group.

$X^0$  to  $X^2$  may be the same or different, and represent a single bond, or an alkylene group, alkenylene group or cycloalkenylene group which may have a substituent,  $-\text{O}-$ ,  $-\text{SO}_2-$ ,  $-\text{O}-\text{CO}-\text{R}^{18}-$ ,  $-\text{CO}-\text{O}-\text{R}^{19}$  or  $-\text{CO}-\text{NR}^{20}-\text{R}^{21}-$ . The alkylene groups  $X^0$  to  $X^2$  may preferably have a substituent. For example, those having 1 to 8 carbon atoms are listed, such as a methylene group, ethylene group, propylene group, butylene group, hexylene group, octylene group and the like. As the alkenylene group, there are preferably listed those having 2 to 6 carbon atoms which may have a substituent, such as an ethenylene group, propenylene group, butenylene group and the like. As the cycloalkylene group, there are preferably listed those having 5 to 8 carbon atoms which may have a substituent, such as a cyclopentylene group, cyclohexylene group and the like. As the alkyl group  $\text{R}^{20}$ , there are listed those having 1 to 4 carbon atoms which may have a substituent, such as a methyl, ethyl group, propyl group, n-butyl group and sec-butyl group. As the cycloalkyl group, there are listed those having 3 to 8 carbon atoms which may have a substituent, such as a cyclopropyl group, cyclopentyl group and cyclohexyl group. As the alkenyl group, there are preferably listed those having 2 to 6 carbon atoms which may have a substituent, such as a vinyl group, propenyl group, allyl group, butenyl group, pentenyl group, hexenyl group and cyclohexenyl group. The alkylene groups, alkenyl groups and cycloalkylene groups  $\text{R}^{18}$ ,  $\text{R}^{19}$  and  $\text{R}^{21}$  include those exemplified above, and further, divalent groups formed by connecting those groups with at least one of ether groups, ester groups, amide groups, urethane groups and ureide groups.

When  $\text{R}^{12}$  to  $\text{R}^{21}$  and  $X^0$  to  $X^2$  have a substituent, the substituent preferably is an alkyl group having 1 to 4 carbon atoms such as a methyl group, ethyl group, propyl group and the like, hydroxyl group, nitro group, further, an alkoxy group having 1 to 8 carbon atoms such as a methoxy group, ethoxy group, propoxy group, butoxy group or the like.

The carboxylic acid generating polymer can be produced by conventionally known various polymerization methods such as radical polymerization, ion polymerization, polycondensation and the like, in the same manner as the sulfonic acid generating polymer. Monomers having a group represented by the formulae (4) to (5) may be polymerized alone or two or more of them may be copolymerized. Further, monomers having a group represented by the formulae (4) to (5) may be copolymerized with the other monomer exemplified for the sulfonic acid generating polymer.

Specific examples of repeating structural units represented by the general formulae (7) to (12) include, but are not limited to, the following units (a1) to (a30).

(a1)



(a2)



(a3)



(a4)



(a5)



(a6)



(a7)



**41**

-continued



(a8)

5



(a9)

15



(a10)

25



(a11)

35



(a12)

45



(a13)

55

60

**42**

-continued



(a14)



(a15)



(a16)



(a17)



(a18)



(a19)



(a20)

-continued



(a21)

(a22) 10

(a23)

(a24)

(a25)

(a26)

(a27)

5

15

20

25

30

35

40

45

50

55

60

-continued

(a28)



(a29)

(a30)



Among above-described carboxylate polymers, those of an alkoxyethyl ester type represented by the structural unit (5) are particularly suitable due to their extremely excellent heat sensitivity.

The polymer having at least one of groups represented by the above-described formulae (1) to (5) used in the present invention has a weight average molecular weight of preferably  $2.0 \times 10^3$  or more, and more preferably in the range from  $5.0 \times 10^3$  to  $3.0 \times 10^5$ . The number-average molecular weight is preferably  $8.0 \times 10^2$  or more, and further preferably in the range from  $1.0 \times 10^3$  to  $2.5 \times 10^5$ . The polydispersibility (weight-average molecular weight/number-average molecular weight) is preferably 1 or more, and more preferably in the range from 1.1 to 10.

These polymer compounds may be in the form of a random polymer, block polymer, graft polymer and the like, and preferably random polymers.

The sulfonic acid generating polymer or carboxylic acid generating polymer used in the present invention may be used alone or in combination. The sulfonic acid generating polymer or carboxylic acid generating polymer can be used in a proportion from 20 to 100% by weight, and preferably

from 50 to 100% by weight based on the total weight of solid components in the heat sensitive layer. If the amount added is less than 20% by weight, sufficient high sensitization may not sometimes be attained.

The layer (b) in the present invention may contain other additives added optionally. For example, the addition of a heat acid generator is preferable in that heat sensitivity is enhanced since decomposition into a sulfonic acid or carboxylic acid is promoted. In the present invention, the heat source which makes layer (b) hydrophilic is layer (c) which can be removed by heat mode, however, depending on occasions, it is possible to add also to a heat sensitive layer a light absorbing agent to act as a supplement for converting irradiated light to heat, for example, an infrared ray absorbing agent may be added when the light source is infrared laser. However, if the amount added thereof is too large, efficient hydrophilization near the substrate which is the effect of the present invention is lost. When an absorbing agent is added, it is preferable that absorbance in relation to the exposure light source is about 0.5 or less.

The heat acid generator added to the layer (b) is one which becomes, after being decomposed by heat, a strong acid which can promote the above-described conversion of a carboxylate to a carboxylic acid or conversion of a sulfonate to a sulfonic acid. An agent which generates by heat decomposition a strong acid manifesting a pKa in water preferably of 4 or less, and more preferably of 2.5 or less is advantageous. For example, any of the groups of compounds usually used as a light acid generator can be used, and in addition, there can be used alkyl esters of organic oxy acids having a pKa of 4 or less, and preferably 3 or less, such as sulfonic acid, phosphoric acid, phosphorous acid, phosphonic acid, boric acid and the like. Use of a heat acid generator having a weight loss temperature (decomposition temperature) calculated by TG/DTA is from 80 to 300° C. is preferable from the viewpoint of storagability and heat decomposability, and more preferably, the weight loss temperature is from 110 to 200° C.

Examples of the compound which generate an acid by heating include, but are not limited to, the following groups of compound. Diazonium salts described in S. I. Schlesinger, Photogr. Sci. Eng., 18, 387 (1974), T. S. Bal et al., Polymer, 21, 423 (1980) and the like, ammonium salts described in U.S. Pat. Nos. 4,069,055, 4,069,056, JP-A No. 3-140,140 and the like, phosphonium salts described in D. C. Necker et al., Macromolecules, 17, 2468 (1984), C. S. wen et al. , Tech, Proc. Conf. Rad. Curing ASIA, p478, Tokyo, Oct (1988), U.S. Pat. Nos. 4,069,055, 4,069,056 and the like, iodonium salts described in J. V. Crivello et al. , Macromolecules, 10 (6), 1307 (1977), Chem. & Eng. News, Nov. 28, p31 (1988), European Patent Application No. 104,143, U.S. Pat. No. 4,837,124, JP-A Nos. 2-150,848, 2-296,514 and the like, sulfonium salts described in J. V. Crivello et al., Polymer J. 17, 73 (1985), J. V. Crivello et al., J. Org. Chem., 43, 3055 (1978), W. R. Watt et al., J. Polymer Sci. , Polymer Chem. Ed., 22, 1789 (1984), J. V. Crivello et al. , Polymer Bull., 14, 279 (1985), J. V. Crivello et al., Macromolecules, 14 (5), 1141 (1981), J. V. Crivello et al. , J. Polymer Sci., Polymer Chem. Ed., 17, 2877 (1979), European Patent Application No. 370, 693, U.S. Pat. No. 3,902,114, European Patent Application Nos. 233,567, 297, 443, 297,442, 422,570, 279,210, U.S. Pat. Nos. 4,933,377, 4,760,013, 4,734,444, 2,833,827, DE Patent Nos. 2,904,626, 3,604,580, 3,604,581 and the like, selenonium salts described in J. V. Crivello et al., Macromolecules, 10 (6), 1307 (1977), J. V. Crivello et al., J. Polymer Sci., Polymer Chem. Ed., 17, 1047 (1979) and the like, onium salts such

as an arsonium salt and the like described in C. S. Wen et al., Tech, Proc. Conf. Rad. Curing ASIA, p478, Tokyo, Oct (1988) and the like, organic halogen compounds described in U.S. Pat. No. 3,905,815, JP-B No. 46-4,605, JP-A Nos. 48-36,281, 55-32,070, 60-239,736, 61-169,835, 61-169,837, 62-58,241, 62-212,401, 63-70,243, 63-298,339 and the like, organometal/organic halogen compounds described in K. Meier et al. , J. Rad. Curing, 13 (4), 26 (1986), T. P. Gill et al., Inorg. Chem., 19, 3007 (1980), D. Astruc, Acc. Chem. Res., 19 (12), 377 (1986), JP-A No. 2-161,445 and the like, photo acid-generating agents having an 0-nitrobenzyl type protecting group described in S. Hayase et al., J. Polymer Sci., 25,753 (1987), E. Reichmanis et al., J. Polymer Sci., Polymer Chem. Ed., 23, 1 (1985), Q. Q. Zhu et al., J. Photochem., 36, 85, 39, 317 (1987), B. Amit et al. , Tetrahedron Lett. , (24) 2205 (1973), D. H. R. Barton et al. , J. Chem. Soc., 3571 (1965), P. M. Collins et al., J. Chem. Soc., Perkin I, 1965 (1975), M. Rudinstei et al., Tetrahedron Lett., (17), 1445 (1975), J. W. Walker et al. , J. Am. Chem. Soc., 110, 7170 (1988), S. C. Busman et al., J. Imaging Technol., 11 (4), 191 (1985), H. M. Houlihan et al., Macromolecules, 21, 2001 (1988), P. M. Collins et al., J. Chem. Soc., Chem. Commun., 532 (1972), S. Hayase et al., Macromolecules, 18, 1799 (1985), E. Reichmanis et al., J. Electrochem. Soc., Solid State Sci. Technol., 130 (6), F. M. Houlihan et al., Macromolecules, 21, 2001 (1988), European Patent Application Nos. 0,290,750, 046,083, 156,535, 271, 851, 0,388,343, U.S. Pat. Nos. 3,901,710, 4,181,531, JP-A Nos. 60-198,538, 53-133,022 and the like, compounds which are photo-decomposed to generate sulfonic acid represented by iminosulfonate and the like described in M. TUNOOKA et al., Polymer Preprints Japan, 35 (8), G. Berner et al. , J. Rad. Curing, 13 (4), W. J. Mijs et al. , Coating Technol., 55 (697), 45 (1983), Akzo, H. Adachi et al., Polymer Preprints, Japan, 37 (3), European Patent Application Nos. 0,199,672, 84,515, 199,672, 044,115, 0,101,122, U.S. Pat. Nos. 4,618,564, 4,371,605, 4,431,774, JP-A Nos. 64-18,143, 2-245,756, 4-365,048 and the like, disulfone compounds described in JP-A No. 61-166,544, o-naphthoquinone diazide-4-sulfonic halides described in JP-A No. 50-36,209 (U.S. Pat. No. 3,969,118), o-naphthoquinone diazide compounds described in JP-A Nos. 55-62,444 (U.K. Patent No. 2,038,801) and JP-B No. 1-11, 935.

In addition to these additives, sulfonates which generate an acid by heat described in Japanese Patent Application Nos. 9-26878, 9-89451, and 9-85328 can be used.

When infrared ray absorbing agents are added to layer (b) the infrared ray absorbing agents are a dye or pigment effectively absorbing an infrared ray having a wavelength of 760 nm to 1,200 nm. It is preferable that the dye or pigment has an absorption maximum between the wavelengths of 760 nm and 1,200 nm.

As dyes, known dyes commercially available or those disclosed in the literature (such as "Senryo Binran (Dye Handbook)" edited by Yuki Gosei Kagaku Kyokai (Organic Synthetic Chemistry Association), published in 1970), can be used. Specifically, examples may include azo dyes, metal complex azo dyes, pyrazolone azo dyes, anthraquinone dyes, phthalocyanine dyes, carbonium dyes, quinoneimine dyes, methyne dyes, cyanine dyes, and metal thiolate complexes.

Examples of preferable dyes may include cyanine dyes disclosed in JP-A Nos. 58-125,246, 59-84,356, 59-202,829, and 60-78,787; methyne dyes disclosed in JP-A Nos. 58-173,696, 58-181,690, and 58-194,595; naphthoquinone dyes disclosed in JP-A Nos. 58-112,793, 58-224,793, 59-48,

187, 59-73,996, 60-52,940, and 60-63,744; squarylium dyes disclosed in JP-A No. 58-112,792; and cyanine dyes disclosed in U.K. Patent No. 434,875.

Furthermore, near infrared absorption sensitizing agents disclosed in U.S. Pat. No. 5,156,938 can be preferably used. Moreover, substituted aryl benzo(thio)pyrylium salts disclosed in U.S. Pat. No. 3,881,924; trimethyne thiapyrylium salts disclosed in JP-A No. 57-142,645 (U.S. Pat. No. 4,327,169); pyrylium-containing compounds disclosed in JP-A Nos. 58-181,051, 58-220,143, 59-41,363, 59-84,248, 59-84,249, 59-146,063, and 59-146,061; cyanine dyes disclosed in JP-A No. 59-216,146; pentamethyne thiopyrylium salts disclosed in U.S. Pat. No. 4,283,475; and pyrylium compounds disclosed in JP-B Nos. 5-13,514 and 5-19,702 can be preferably used as well.

As other examples of preferable dyes, near infrared absorption dyes disclosed in U.S. Pat. No. 4,756,993 represented by formulas (I) and (II) can be presented.

Among these dyes, particularly preferable are cyanine dyes, squarylium dyes, pyrylium salts, and nickel thiolate complexes.

Pigments usable in the present invention may include commercially available pigments and those disclosed in the Color Index (C. I.) Manual, "Saishin Ganryo Binran (Modern Pigment Manual)" edited by Nippon Ganryo Gijutsu Kyokai (Japan Pigment Technology Association), published in 1977; "Saishin Ganryo Oyo Gijutsu (Modern Pigment Application Technology)" by CMC Press, published in 1986; and "Insatsu Ink Gijutsu (Printing Ink Technology)" by CMC Press, published in 1984.

Examples of pigments may include black pigments, yellow pigments, orange pigments, brown pigments, red pigments, purple pigments, blue pigments, green pigments, fluorescent pigments, metal powder pigments, and polymer bond pigments. Specifically, insoluble azo pigments, azo lake pigments, condensation azo pigments, chelate azo pigment, phthalocyanine pigments, anthraquinone pigments, perylene and perynone pigments, thioindigo pigments, quinacridone pigments, dioxazine pigments, isoindolinone pigments, quinophthalone pigments, colored lake pigments, azine pigments, nitroso pigments, nitro pigments, natural pigments, fluorescent pigments, inorganic pigments, and carbon black can be used. Among these examples, carbon black is preferable.

These pigments can be used without surface treatment, or can be used after the application of a surface treatment.

Examples of surface treatment methods may include a method of surface coating with a resin or a wax, a method of adhering a surfactant thereto, and a method of bonding a reactive substance (such as a silane coupling agent, an epoxy compound, or a polyisocyanate) with the pigment surface. The above-mentioned surface treatment methods are disclosed in "Kinzokusekken no Seishitsu to Oyo (Natures and Applications of Metal Soaps)" by Sachi Press; "Insatsu Ink Gijutsu (Printing Ink Technology)" by CMC Press; published in 1984; and "Saishin Ganryo Oyo Gijutsu (Modern Pigment Application Technology)" by CMC Press, published in 1986.

A pigment particle size of  $0.01 \mu\text{m}$  to  $10 \mu\text{m}$  is preferable,  $0.05 \mu\text{m}$  to  $1 \mu\text{m}$  is more preferable, and  $0.1 \mu\text{m}$  to  $1 \mu\text{m}$  is the most preferable. A pigment particle size smaller than  $0.01 \mu\text{m}$  is not preferable in terms of the stability of the pigment dispersion in a photosensitive layer coating solution. On the other hand, a pigment particle size larger than  $10 \mu\text{m}$  is not preferable in terms of the uniformity of the image recording layer.

As methods of dispersing a pigment, known dispersing methods employed in ink production or toner production can

be used. Examples of the dispersing machine include ultrasonic dispersing machines, sand mills, attritors, pearl mills, super mills, ball mills, impellers, dispersers, KD mills, colloid mills, dynatrons, triple roll mills, and pressure kneaders. Details thereof are described in "Saishin Ganryo Oyo Gijutsu (Modern Pigment Application Technology)" by CMC Press, published in 1986.

These dyes or pigments can be added to an image recording material in an amount of 0.01 to 50% by weight based on the weight of the total solid component of the image recording material, preferably in an amount of 0.1 to 10% by weight, and more preferably in an amount of 0.5 to 10% by weight in the case of a dye, and more preferably in an amount of 3.1 to 10% by weight in the case of a pigment. An amount of a pigment or dye less than 0.01% by weight causes low sensitivity. On the other hand, an amount more than 50% by weight produces stains in nonimage portions at the time of printing.

In the present invention, other additives may further be added to layer (b) according to necessity. For example, a dye having a large absorption in the visible light region can be added as a coloring agent. Specifically, examples may include Oil Yellow #101, Oil Yellow #103, Oil Pink #312, Oil Green BG, Oil Blue BOS, Oil Blue #603, Oil Black BY, Oil Black BS, Oil Black T-505 (manufactured by Orient Chemical Industry, Co., Ltd.), Victoria Pure Blue, Crystal Violet (CI42555), Methyl Violet (CI42535), Ethyl Violet, Rhodamine B (CI145170B), Malachite Green (CI42000), Methylene Blue (CI52015), and dyes disclosed in JP-A No. 62-293,247.

In order to guarantee stable treatment regardless of fluctuations in the printing conditions, a nonionic surfactant disclosed in JP-A Nos. 62-251,740 and 3-208,514 and an ampholytic surfactant disclosed in JP-A Nos. 59-121,044 and 4-13,149 can be added to layer (b) of the present invention.

Examples of nonionic surfactants may include sorbitan tristearate, sorbitan monopalmitate, sorbitan triolate, mono glyceride stearate, and polyoxyethylene nonylphenyl ether.

Examples of ampholytic surfactants may include alkyl di(aminoethyl)glycine, alkyl polyaminoethylglycine hydrochloride, 2-alkyl-N-carboxyethyl-N-hydroxyethyl imidazolinium betaine, and N-tetradecyl-N,N-substituted betaine (for example, Amorgen K manufactured by Dai-Ichi Kogyo Co., Ltd.).

The amount of the above-described nonionic surfactants and ampholytic surfactants is preferably from 0.05 to 15% by weight, and more preferably from 0.1 to 5% by weight in an image recording material.

In order to provide flexibility to the film, etc., a plasticizer can be added as needed to layer (b) of the present invention. Examples of a plasticizer may include polyethylene glycol, tributyl citrate, diethyl phthalate, dibutyl phthalate, dihexyl phthalate, dioctyl phthalate, tricresyl phosphate, tributyl phosphate, trioctyl phosphate, tetrahydrofurfuryl oleate, an oligomer and a polymer of acrylic acid or methacrylic acid.

In addition to these examples, epoxy compounds, vinyl ethers, phenol compounds having an alkoxy methyl group and phenol compounds having a hydroxymethyl group disclosed in Japanese Patent Application No. 7-18,120, can also be added. Other polymer compounds can be added in order to increase the strength of the film.

The planographic printing plate of the present invention can be produced, in general, by dissolving the above-described component in a solvent and applying the resultant solution to an appropriate support. Solvents used herein may include, but are not limited to, ethylene dichloride,

cyclohexanone, methyl ethyl ketone, methanol, ethanol, propanol, ethylene glycol monomethyl ether, 1-methoxy-2-propanol, 2-methoxy ethyl acetate, 1-methoxy-2-propyl acetate, dimethoxyethane, methyl lactate, ethyl lactate, N,N-dimethyl acetamide, N,N-dimethyl formamide, tetramethyl urea, N-methyl pyrrolidone, dimethyl sulfoxide, sulfolane,  $\gamma$ -butyrolactone, toluene and water.

These solvents are used alone or in combinations thereof. The concentration of the above-described components (total solid component including additives) is preferably from 1 to 50% by weight in the solution.

A surfactant for improving the applicability, such as a fluorine-containing surfactant disclosed in JP-A No. 62-170, 950 can be added to layer (b) of the present invention. The amount added is preferably from 0.01 to 1% by weight based on the total solid component of the image recording material, and more preferably from 0.05 to 0.5% by weight.

The amount coated of layer (b) obtained after coating and drying (solid component) differs depending on use, and in the case of the printing plate precursor (1), 0.5 to 5.0 g/m<sup>2</sup> is preferable and 0.5 to 1.5 g/m<sup>2</sup> is more preferable. In the present invention since layer (b) is coated after the formation of layer (a) and both of them are partially compatibilized at the interface, adhesion between hydrophilic layer (a) and hydrophobic layer (b) becomes excellent and releasing between the layers is effectively prevented.

The amount coated of layer (b) (solid component) in the printing plate precursors (2) and (3) differs depending on the overall structure of the printing plate precursor, and in general, is preferably 2.0 g/m<sup>2</sup> or less, and more preferably 1.0 g/m<sup>2</sup> or less. For conducting coating, various methods can be used, and for example, bar coater coating, rotation coating, spray coating, curtain coating, dip coating, air knife coating, blade coating, roll coating, and the like are listed.

#### Layer (c)

In the present invention, the phrase "removal by heat mode exposure" neither means that all recording layer components disappear in the stage of irradiation in the irradiation range nor means that substantial reduction in weight necessarily accompanies the irradiation stage. The phenomenon caused by the irradiation is characterized in that form change in the form of the recording layer solid follows, and it means that the structure of the layer is substantially decomposed. Scientifically, phenomena such as ablation, evaporation, melting and the like are included, and these are not necessarily accompanied by a reduction in weight. However, such a form change in the present invention is required to cause at least partial removal of irradiation portions in the intermediate layer, in some cases in the irradiation stage, and in other cases in post treatment or printing process. Such form change can be recognized by various microscopic means, and the recording layer in the present invention is required to be able to cause at least such a form change.

Any hydrophilic solid thin layer or organic thin layer which can absorb irradiated light can be suitably used in layer (c) in the planographic printing plate precursor of the present invention, and any known materials in this field, and the fields of metal processing, laser processing and the like can be used. The preferable layer (c) is generally one whose absorbance is as high as possible and whose thickness is as thin as possible, in view of the printing ability and image forming speed (sensitivity). When absorbance of irradiated light is low, the sensitivity decreases since the amount of heat generation due to light-to-heat conversion is low. When the film thickness is high, the sensitivity decreases because of the large amount of heat required for the removal or the

removal becomes completely impossible, thereby causing blemishes in printing. The preferable absorbance is 0.1 or more, more preferably 0.5 or more, and most preferably 1.0 or more. The preferable thickness largely depends on the components of the layer (c) and when the layer (c) is an inorganic solid thin film (metal film and the like) described below, it is preferably 5000 Å or less, and more preferably 1000 Å or less, and in the case of an organic thin film, it is preferable that the amount coated is 500 mg/m<sup>2</sup> or less, and more preferably 100 mg/m<sup>2</sup> or less. The lower limit of the film thickness depends on absorbance, and the preferable thickness may advantageously be determined so that absorbance is 0.1 or more.

As the solid thin film, various inorganic solid thin films can be used described for example in JP-A Nos. 55-113307 and 52-37104. Specifically, for example, Mg, Sc, Y, Ti, Zr, Hf, V, Nb, Ta, Cr, Mo, W, Mn, Re, Fe, Co, Ni, Ru, Rh, Pd, Ir, Pt, Cu, Ag, Au, Zn, Cd, Al, Ga, In, Si, Ge, Pb, Sn, As, Sb, Bi, Se, Te, and the like are listed, and among these, Mg, Ti, Cr, Cu, Ag, Zn, Al, In, Sn, Bi, and Te are particularly advantageous in view of their sensitivity. In addition, there can be also used thin alloy films composed of compounds obtained by optionally changing the oxidation condition of the above-described metals (oxygen compounds, nitrogen compounds, and the like), stainless steel, brass and the like, chalcogen materials (S, Se simple substances, and the like), binary chalcogen materials (As—S system, As—Se system, As—Te system, S—Se system, Sb—Se system, Sb—Te system, Bi—S system, Bi—Se system, Bi—Te system, Ge—S system, Sn—S system, and the like), ternary chalcogen materials (As—S—Te system, As—Se—Te system, Ge—Sn—S system, and the like), graphite and the like, and further, inorganic thin films prepared by modifying these materials by oxidation, doping, and the like according to necessity can also be used. These thin films can be formed by usual methods such as dry methods such as vapor deposition (resistance heating, electron beam and the like), sputtering and ion plating on a substrate, and wet coating methods such as a method using electrochemical depositing, a sol gel method and the like, and in addition, the thin film can be formed for example, by a silver halide emulsion layer diffusion transfer developing method, however, the effect of the present invention is not limited by these film forming methods.

When an organic thin film is used as layer (c), the organic thin layer contains a suitable light absorbing agent. The organic thin film is usually constituted of a binder resin having film forming ability and a light absorbing agent, and optionally, a compound obtained by chemically binding these two components may also be used.

As the binder resin used in the organic thin film, those widely and generally known can be used without particular restriction. Specifically, novolak resins (phenol-formaldehyde resin, cresol-formaldehyde resin and the like), urea-formaldehyde resins, melamine-formaldehyde resins, alkyd resins, (meth)acrylic resins (polymethyl methacrylate, polyethyl acrylate and the like), styrene-based resins (polystyrene,  $\alpha$ -methylpolystyrene and the like), polyamide-based resins (nylons), polyester resins, polyurethane-based resins, polyurea-based resins, polycarbonate resins, silicone-based resins, esters of polyvinylacetal (polyvinyl acetate and the like), acetals of polyvinyl alcohol (polyvinylboryral and the like), vinyl-based resin (polyvinyl chloride and the like), polyalkenes (polyethylene and the like) styrene-butadiene resins, polyvinylidene chlorides, fluorine-based resins, poly-organosiloxanes (polydimethylsiloxane and the like), organism polymer modified materials (polysaccharide,

oligosaccharide, polypeptide and the like) and modified materials thereof (cellulose acetate, cellulose acetate butyrate and the like).

As the light absorbing agent used in the organic thin film, compounds which can absorb light energy radiation used for recording can be used without limitation. In the production of a printing plate using infrared laser which is a preferable embodiment of the present invention, it is desirable that the above-described light absorbing agent is an infrared absorbing agent. As examples of preferable infrared ray absorbing agents, those previously exemplified for the additive to layer (b) may be listed.

For producing the layer (c) when layer (c) is an organic thin film, the same methods used for the above-described layer (b) are listed. In general, layer (c) can be produced by dissolving components in a solvent and coating the mixture on a suitable substrate. Examples of the solvent herein used include, but are not limited to, ethylene dichloride, cyclohexanone, methyl ethyl ketone, methanol, ethanol, propanol, ethylene glycol monomethyl ether, 1-methoxy-2-propanol, 2-methoxyethyl acetate, 1-methoxy-2-propyl acetate, dimethoxyethane, methyl lactate, ethyl lactate, N,N-dimethylacetamide, N,N-dimethylformamide, tetramethylurea, N-methylpyrrolidone, dimethylsulfoxide, sulfolane, Y-butyrolactone, toluene, water and the like.

These solvents are used alone or in combination. The concentration of the above-described components (total solid components in layer (c) including additives) in the solvent is preferably from 1 to 50% by weight. The amount coated (solid components) on a substrate obtained after coating and drying is not particularly restricted, and in general, is preferably from 0.2 to 3.0 g/m<sup>2</sup>. For conducting coating, various methods can be used, and for example, bar coater coating, rotation coating, spray coating, curtain coating, dip coating, air knife coating, blade coating, roll coating and the like are listed.

To the intermediate layer in the present invention, a surfactant for improving coatability, for example, fluorine-based surfactants as described in JP-A No. 62-170950 can be added. The amount added thereof is preferably from 0.01 to 1% by weight, and more preferably from 0.05 to 0.5% by weight based on the total weight of the solid components in the image recording material.

It is known that among the above-described general structures which cause form change by heat mode exposure and become substantially removable, use of specific materials and structure is advantageous from the viewpoint of recording sensitivity. Such known technology can be utilized also in the present invention without exception. For example, use or addition of a self-oxidizing resin such as nitrocellulose and the like described in JP-A No. 49-117102 (U.S. Pat. No. A86656) and U.S. Pat. No. 3,962,513 is suitable in that recording sensitivity is enhanced. Acrylic cross-linked polymers described in U.S. Pat. No. 3,574,657 have high sensitivity and are thus suitable. Further, the sensitivity is relatively improved also by the use of heat-decomposable resins of polyesters, polymethyl methacrylates, and polyoxymethylenes described in U.S. Pat. No. 4,054,094. WO90-01635 and 94-01280 describe a group of polymers excellent in heat-decomposability, and any of these are suitable from the viewpoint of sensitivity. The sensitivity can be improved by the addition of halogen, Ge, Si and the like to a chalcogen-based recording layer, or by the addition, as a constituting component, of an alkaline metal such as Na, K and the like, an alkaline earth metal such as Ca, Sr, and the like, a IVb group element such as Si, Ge, Sn, Pb, and the like, a IIIb group element such as Tl, Al, In,

and the like, a IIb group element such as Zn and the like, a lanthanum-based rare earth element such as Eu, Sm, and the like, an actinide rare earth element such as U and the like, as well as other elements, as described in JP-A No. 50-11307. As described in JP-A No. 52-37140, used of an aluminum substrate having an anodized coating of 0.5 μm or more is advantageous from the viewpoint of heat scattering. Addition of compounds (CrS, Cr<sub>2</sub>S, Cr<sub>2</sub>S<sub>3</sub>, MoS<sub>2</sub>, MnS, FeS, FeS<sub>2</sub>, CoS, Co<sub>2</sub>S<sub>3</sub>, NiS, Ni<sub>2</sub>S, PbS, Cu<sub>2</sub>S, Ag<sub>2</sub>S, ZnS, In<sub>2</sub>S<sub>3</sub>, GeS<sub>x</sub> (wherein, x represents a positive integer), SnS, SnS<sub>2</sub>, PbS, As<sub>2</sub>S<sub>3</sub>, Sb<sub>2</sub>S<sub>3</sub>, Bi<sub>2</sub>S<sub>2</sub>, MgF<sub>2</sub>, CaF<sub>2</sub>, RhF<sub>3</sub>, MoO, InO, In<sub>2</sub>O, In<sub>2</sub>O<sub>3</sub>, GeO, PbO) to a metal recording layer which is deformed by heating, or making the metal recording layer into a multi-layer structure as described in JP-A No. 53-33702 is effective for high sensitization. When a light absorbing agent is combined with a halogen-containing polymer as disclosed in JP-A No. 62-9993, sensitivity preferably increases. Further, a recording layer mainly composed of a light absorbing agent, thermoplastic resin and a lower molecular weight compound soluble in an organic solvent as disclosed in JP-A No. 5-138848 is advantageous from the viewpoints of recording sensitivity and blemishability of a print. When cyanoacrylate polymers (poly(methyl-2-cyanoacrylate), poly(methyl-2-cyanoacrylate-2-ethyl-2-cyanoacrylate), poly(methoxyethyl-2-cyanoacrylate), and the like) are used as a binder as described in U.S. Pat. No. 5,605,780, a planographic plate precursor excellent in printability having relatively high sensitivity is obtained since the binder is excellent in heat decompability.

An additive for improving the various properties thereof as a printing plate precursor may be added to layer (c). As preferable examples of the additive, the above-described heat acid generators, coloring agents, surfactants, plasticizers and the like exemplified for layer (b) are listed.

The substrate will now be described.

The substrate used in the planographic printing plate precursor of the present invention has at least a surface which is hydrophilic. As such a substrate, conventionally known hydrophilic substrates used for planographic printing plates can be used without limitation. The substrate used is preferably a dimensionally stable plate material, and examples thereof include paper, paper laminated with a plastic (for example, polyethylene, polypropylene, polystyrene or the like) metal plates (for example, aluminum, zinc, copper and the like) plastic films (for example, cellulose diacetate, cellulose triacetate, cellulose propionate, cellulose butyrate, cellulose acetate butyrate, cellulose nitrate, polyethylene terephthalate, polyethylene, polystyrene, polypropylene, polycarbonate, polyvinylacetal and the like), paper and plastic films laminated or deposited with the above-described metals, and the like, and suitable known physical or chemical treatments may be optionally performed on the surface of these substrates for the purpose of imparting hydrophilicity, increasing strength and the like.

In particular, as preferable substrates, paper, polyester films or aluminum plates are listed, and among these, particularly preferable is an aluminum plate which has excellent dimensional stability, is relatively cheap, and can provide a surface excellent in hydrophilicity and strength through surface treatment according to demands. Further, a complex sheet prepared by bonding an aluminum sheet on a polyethylene terephthalate film is also preferable as described in JP-B No. 48-18327. As the aluminum plate, a pure aluminum sheet, and alloy plates mainly composed of aluminum and containing a small amount of hetero atoms are suitably used, and further, plastic films on which alumi-

num is laminated or deposited are permissible. Examples of the hetero atoms contained in the aluminum alloy include silicon, iron, manganese, copper, magnesium, chromium, zinc, bismuth, nickel, titanium and the like. The content of hetero elements in the alloy is at most 10% by weight. In the present invention, particularly preferable aluminum is pure aluminum, however, it is difficult to produce completely pure aluminum due to refining technology, therefore, aluminum containing a slight amount of hetero elements may also be allowable. Thus, the composition of the aluminum plate used in the present invention is not specified, and an aluminum plate composed of conventionally known and used materials can be appropriately utilized. The thickness of the aluminum plate used in the present invention is from about 0.1 mm to 0.6 mm, preferably from 0.15 mm to 0.4 mm, and particularly preferably from 0.2 mm to 0.3 mm.

In the case of a substrate having a metal surface, in particular an aluminum surface, it is preferable that a surface treatment such as a roughening (graining) treatment, immersion treatment in an aqueous solution of sodium silicate, potassium fluorinated zirconate, phosphate salt and the like, or an anodizing treatment is performed.

The roughening treatment of the surface of an aluminum plate is conducted by various methods, for example, a mechanical roughening method, a method for electrochemically dissolving and roughening the surface, and a method for selectively dissolving the surface chemically. As mechanical methods, known methods can be used such as a ball grinding method, brush grinding method, blast grinding method, buffing grinding method and the like. As electrochemical roughening methods, there are methods using alternating current or direct current in an electrolyte solution such as hydrochloric acid, nitric acid and the like. Also, a method combining both means can be used as disclosed in JP-A No. 54-63902. Prior to the roughening of an aluminum plate, if desired, there maybe conducted, for example, a degreasing treatment using a surfactant, organic solvent or alkaline aqueous solution for removing rolling oil on the surface.

Further, there is preferably used an aluminum plate which is, after roughening treatment, subjected to immersion treatment in an aqueous sodium silicate solution. As described in JP-B No. 47-5125, an aluminum plate is suitably used which is subjected to anodizing treatment, then, immersed into an aqueous solution of an alkaline metal silicate. The anodizing treatment is carried out by applying current using aluminum as an anode in an electrolyte solution composed solely of, for example, an aqueous solution or non-aqueous solution of an inorganic acid such as phosphoric acid, chromic acid, sulfuric acid, boric acid and the like, or an inorganic acid such as oxalic acid, sulfamic acid and the like, or salts thereof, or composed of a combination of two or more of these.

Further, silicate electric deposition as described in U.S. Pat. No. 3,658,662 is also effective.

Further, surface treatment combining a substrate on which an electrolytic grain is applied, the above-described anodizing treatment and sodium silicate treatment is also useful as disclosed in JP-B No. 46-27481 and JP-A Nos. 52-58602 and 52-30503.

As disclosed in JP-A No. 56-28893, a substrate which is subjected to mechanical roughening, chemical etching, electrolytic grain, anodizing treatment and sodium silicate treatment in sequence is also suitable.

Further, a substrate on which a water-soluble resin, for example, a polymer and copolymer containing as the side chain a polyvinylphosphonate group or sulfonate group,

polyacrylic acid, water-soluble metal salt (for example, zinc borate) or yellow dye, amine salt and the like is applied as a primer, after the above-described treatments, is also suitable.

As disclosed in Japanese Patent Application No. 5-304358, there is also suitably used a sol-gel treated substrate on which a functional group which may cause addition reaction by radical is bonded by covalent linkage.

As other preferable examples, there are also listed those prepared by providing a water resistant hydrophilic layer as the surface layer on any substrate. As such a surface layer, there are listed, for example, layers composed of an inorganic pigment and a bonding agent described in U.S. Pat. No. 305,295 and JP-A No. 56-13168, a hydrophilic swelling layer described in JP-A No. 9-80744, and a sol-gel film composed of titanium oxide, polyvinyl alcohol and silicic acids described in Japanese Patent Application National Publication (Laid-Open) No. 8-507727.

The planographic printing plate precursor of the present invention is produced in the manner described above. In particular, a method is preferable in which an image is exposed by a solid laser or semiconductor laser which emits an infrared ray having a wavelength of 700 nm to 1200 nm to produce a plate. In the present invention, the printing plate may be installed in a printing machine immediately after image exposure and printing may be conducted, however, if necessary, it is also possible that the printing plate precursor is previously installed in a printing machine and image exposure is conducted on the printing machine and printing is conducted in such a condition. Production of a printing plate in this way is preferable since the production process can be simplified. However, between the image exposure process and the printing process, there may be conducted post treatment processes such as washing of the surface of a recording layer and post heating, if necessary. By these processes, it becomes possible to further improve the resistance to blemishing of non-image portions, strengthen image portions, improve printing durability and scratch resistance, and decrease the exposure time necessary for image exposure, or maintain desirable surface properties of a planographic printing plate after image exposure for a longer period of time.

The planographic printing plate precursor (1) having undergone image exposure can be developed with water after the exposure, subjected to gum coating if necessary, then, installed in a printing machine for conducting printing, and further, can also be installed in a printing machine immediately after exposure (without a developing process) to conduct printing. Namely, in the plate production method using the planographic printing plate precursor of the present invention, a planographic printing plate can be produced without a particular developing treatment. The water development in the present invention indicates development using a developing solution having a pH of 2 or more composed of water or mainly composed of water.

The planographic printing plate obtained by such treatment is applied to an offset printing machine, and used for printing for providing a large number of prints.

## EXAMPLES

The following examples further illustrate the present invention in detail below, but do not limit the scope thereof. Preparation of Substrate

An aluminum plate (material 1050) having a thickness of 0.30 mm was degreased by washing with trichloroethylene. A roughening treatment was applied to the aluminum plate by graining the surface with a nylon brush and a suspension

55

in which a 400 mesh powder of pumice stone was suspended in water. The plate was then washed with water. The plate was etched by being immersed in a 25% aqueous solution of sodium hydroxide at 45° C. for 9 seconds and washed with water. The plate was further immersed in a 2%  $\text{HNO}_3$  for 20 seconds and washed with water. The etching amount of the grained surface was about 3 g/m<sup>2</sup>. Then, the plate was provided with a direct current anodic oxidization film of about 3 g/m<sup>2</sup> with 7%  $\text{H}_2\text{SO}_4$  as the electrolyte and a current density of 15 A/dm<sup>2</sup>, washed with water, and dried. The resulting substrate was named S-1. The contact angle against a water drop in air of S-1 was 100 or less.

Example of planographic printing plate (1)

Synthesis of hydrophilic polymer compound

0.5 g of benzoyl peroxide was added as a polymerization initiator to 60 g of vinyl acetate and 40 g of methyl acrylate, and the resulting mixture was dispersed in 300 ml of water containing 3 g of a partially saponified polyvinyl alcohol and 10 g of NaCl as dispersing stabilizers.

The dispersion was stirred for 6 hours at 65° C. to conduct suspension polymerization. The content of the methyl acrylate component in the resulting copolymer was identified by NMR spectrum at 48 mol %. The intrinsic viscosity in a benzene solution at 30° C. was 2.10.

Then 8.6 g of this copolymer was added to a saponification reaction solution composed of 200 g of methanol, 10 g of water and 40 ml of 5N NaOH and the mixture was stirred in suspension, saponification reaction was conducted at 25° C. for 1 hour, then, the temperature was increased to 65° C. and further saponification reaction was conducted for 5 hours.

The resulting saponification reaction product was washed fully with methanol, and freeze-dried. The degree of saponification was 98.3 mol %, and it was verified as a result of infrared spectrum measurement that strong absorption derived from —COO— group was 1570 cm<sup>-1</sup>.

Synthesis of heat sensitive polymer compound

Synthesis of monomer (4)

200 ml of acetonitrile, 11 g of cyclohexyl alcohol and 8.8 g of pyridine were charged into a 500 ml three-necked flask, and stirred. To this was added 20.2 g of vinylbenzenesulfonyl chloride dropwise while being cooled with ice. After completion of the addition, the mixture was stirred for 2 hours, then, poured into 1 liter of water and extracted with ethyl acetate. The product was dried over magnesium sulfate, then the solvent was distilled under reduced pressure, and the residue was purified by column chromatography on silica gel to obtain a monomer (4). Element Analysis: the calculated values were; C: 63.13%, H: 6.81%, the actual values were; C: 63.01%, H: 6.85%

Synthesis of monomer (5)

A monomer (5) was synthesized in the same manner as for the monomer (4) except that 2,2,2-trifluoroethyl alcohol was used instead of cyclohexyl alcohol.

Synthesis of monomer (10)

A monomer (10) was synthesized in the same manner as for the monomer (4) except that the alcohol described below was used instead of cyclohexyl alcohol.

56



10 Synthesis of monomer (49)

1.06 g of 2,4-dinitrotoluene, then 500 g of methacrylic acid and 488 g of dihydropyran were charged into a 500 ml three-necked flask. To this mixture was added concentrated hydrochloric acid while being cooled with ice. After 15 completion of the addition, the reaction mixture was warmed to about 60° C. and stirring was continued for 2 hours and 30 minutes at the same temperature. The reaction mixture was cooled to room temperature, and the reaction mixture was changed to alkaline with an aqueous sodium hydroxide solution. From this mixture, product was extracted with ethyl acetate, and the organic layer was dried over magnesium sulfate then concentrated under reduced pressure. The resulting solution was verified by identification by NMR that: monomer (49): 88.1% by weight, ethyl acetate: 12.9% by weight.

25 Synthesis of heat sensitive polymer compound (1)

20 g of the monomer (4) and 40 g of methyl ethyl ketone were charged into a 200 ml three-necked flask, and to this was added 0.25 g of azobisisdimethylvaleronitrile at 65° C. under nitrogen flow. This temperature was maintained for 5 hours while being stirred, then the solvent was distilled off under reduced pressure, to obtain a solid material. By GPC, it was verified as a polymer having a weight-average molecular weight of 15200.

30 Synthesis of heat sensitive polymer compounds (2) to (4)

35 Heat sensitive polymer compounds (2) to (4) were synthesized in the same manner as for the heat sensitive polymer compound (1) except the raw material monomer (4) was changed for the monomers shown in the following Table 1. The average molecular weights of the resulting polymers are shown in the following Table 1.

TABLE 1

|                                     | Monomer used | Weight-average molecular weight |
|-------------------------------------|--------------|---------------------------------|
| Heat sensitive polymer compound (2) | Monomer (5)  | 20 g 16000                      |
| Heat sensitive polymer compound (3) | Monomer (10) | 20 g 18000                      |
| Heat sensitive polymer compound (4) | Monomer (49) | 20 g 20000                      |

45 Synthesis of heat sensitive polymer compound (5)

50 7.18 g of the monomer (4), 0.31 g of ethyl acrylate and 15 g of methyl ethyl ketone were charged into a 100 ml three-necked flask, and to this was added 0.1 g of azobisisdimethylvaleronitrile at 65° C. under nitrogen flow. The mixture was stirred for 5 hours at the same temperature, then, the methyl ethyl ketone was distilled off under reduced pressure, to obtain a solid material. By GPC (polystyrene standard), it was recognized as a polymer having a weight-average molecular weight of 18000.

55 Synthesis of heat sensitive polymer compounds (6) to (8)

60 Heat sensitive polymer compounds (6) to (8) were synthesized in the same manner as for the heat sensitive polymer compound (5) except the raw material monomer (4) was replaced by the monomers shown in the following Table

2. The average molecular weights of the resulting polymers are shown in the following Table 2.

TABLE 2

|                                     | Monomer used | Weight-average molecular weight |
|-------------------------------------|--------------|---------------------------------|
| Heat sensitive polymer compound (6) | Monomer (5)  | 7.18 g 16000                    |
| Heat sensitive polymer compound (7) | Monomer (10) | 9.05 g 18000                    |
| Heat sensitive polymer compound (8) | Monomer (49) | 4.59 g 25000                    |

## Examples 1 to 9

The following solution [A] was coated on the above-described substrate S-1, and dried for 2 minutes at 100° C. to obtain an aluminum plate coated with a layer (a). The weight after drying was 1.1 g/m<sup>2</sup>.

| Solution [A]                                                                                            |        |
|---------------------------------------------------------------------------------------------------------|--------|
| Hydrophilic polymer compound                                                                            | 1.0 g  |
| Fluorine-based surfactant (trade name: Megafack F-177, manufactured by Dainippon Ink & Chemicals, Inc.) | 0.06 g |
| Methyl alcohol                                                                                          | 5.0 g  |
| Purified water (Only to [B-9], dye 1                                                                    | 0.08 g |

Nine solutions [B-1] to [B-9] were prepared by changing the type of heat sensitive polymer compound in the following solution [B] as is shown in Table 3. The resulting solutions were respectively coated on the above-described aluminum plate coated with layer (a), and dried at 80° C. for 3 minutes to obtain planographic printing plate precursors [B-1] to [B-9]. The weight after drying was 1.2 g/m<sup>2</sup>.

| Solution [B]                                                                                |        |
|---------------------------------------------------------------------------------------------|--------|
| Heat sensitive polymer compound (Table 3)                                                   | 4.0 g  |
| Infrared ray absorbing agent (IR-125, manufactured by Wako Pure Chemical Industries Ltd.)   | 0.15 g |
| Acid generator: Salt of diphenyliodoniumanthraquinonesulfonic acid                          | 0.15 g |
| Dye in which counter ion in Victoria Pure Blue BOH is changed to 1-naphthalenesulfonic acid | 0.05 g |
| Fluorine-based surfactant (Megafack F-177, manufactured by Dainippon Ink & Chemicals, Inc.) | 0.06 g |
| Methyl ethyl ketone                                                                         | 20 g   |
| γ-Butyrolactone                                                                             | 10 g   |
| 1-Methoxy-2-propanol                                                                        | 8 g    |
| Water                                                                                       | 2 g    |

TABLE 3

|           | Planographic printing plate precursor | Heat sensitive polymer compound |
|-----------|---------------------------------------|---------------------------------|
| Example 1 | [B-1]                                 | (1)                             |
| Example 2 | [B-2]                                 | (2)                             |
| Example 3 | [B-3]                                 | (3)                             |
| Example 4 | [B-4]                                 | (4)                             |
| Example 5 | [B-5]                                 | (5)                             |

TABLE 3-continued

|           | Planographic printing plate precursor | Heat sensitive polymer compound |
|-----------|---------------------------------------|---------------------------------|
| Example 6 | [B-6]                                 | (6)                             |
| Example 7 | [B-7]                                 | (7)                             |
| Example 8 | [B-8]                                 | (8)                             |
| Example 9 | [B-9]                                 | (1)                             |

The resulting planographic printing plate precursors [B-1] to [B-9] were exposed by YAG laser emitting an infrared ray having a wavelength of 1064 nm at laser power: 360 mW and scanning speed: 3.0 m/s. After the exposure, they were heated at 110° C. for 1 minute, then printed using a Hydel KOR-D Machine. In this procedure, it was observed whether blemishes occurred on non-image portions of the print or not. The results are shown in Table 4.

TABLE 4

|           | Planographic printing plate precursor | Blemishes on non-image portions in printing |
|-----------|---------------------------------------|---------------------------------------------|
| Example 1 | [B-1]                                 | None                                        |
| Example 2 | [B-2]                                 | None                                        |
| Example 3 | [B-3]                                 | None                                        |
| Example 4 | [B-4]                                 | None                                        |
| Example 5 | [B-5]                                 | None                                        |
| Example 6 | [B-6]                                 | None                                        |
| Example 7 | [B-7]                                 | None                                        |
| Example 8 | [B-8]                                 | None                                        |
| Example 9 | [B-9]                                 | None                                        |

As is apparent from the results of Table 4, according to the planographic printing plate of the present invention, excellent prints having no blemishes on non-image portions were obtained even at the low energy exposure of a 3.0 m/s scanning speed.

## Comparative Examples 1 to 8

Eight solutions [C-1] to [C-8] were prepared by changing the type of heat sensitive polymer compound in the following solution [C]. The resulting solutions were respectively coated on the above-described aluminum plate S-1 treated as described above, and dried at 100° C. for 2 minutes to obtain planographic printing plate precursors [C-1] to [C-8]. The weight after drying was 1.2 g/m<sup>2</sup>.

| Solution [C]                                                                                |        |
|---------------------------------------------------------------------------------------------|--------|
| Heat sensitive polymer compound (Table 5)                                                   | 4.0 g  |
| Infrared ray absorbing agent (IR-125, manufactured by Wako Pure Chemical Industries Ltd.)   | 0.15 g |
| Acid generator: Salt of diphenyliodoniumanthraquinonesulfonic acid                          | 0.15 g |
| Dye in which counter ion in Victoria Pure Blue BOH is changed to 1-naphthalenesulfonic acid | 0.05 g |
| Fluorine-based surfactant (Megafack F-177, manufactured by Dainippon Ink & Chemicals, Inc.) | 0.06 g |
| Methyl ethyl ketone                                                                         | 20 g   |
| γ-Butyrolactone                                                                             | 10 g   |
| 1-Methoxy-2-propanol                                                                        | 8 g    |
| Water                                                                                       | 2 g    |

TABLE 5

|                       | Planographic printing plate precursor | Heat sensitive polymer compound |
|-----------------------|---------------------------------------|---------------------------------|
| Comparative example 1 | [C-1]                                 | (1)                             |
| Comparative example 2 | [C-2]                                 | (2)                             |
| Comparative example 3 | [C-3]                                 | (3)                             |
| Comparative example 4 | [C-4]                                 | (4)                             |
| Comparative example 5 | [C-5]                                 | (5)                             |
| Comparative example 6 | [C-6]                                 | (6)                             |
| Comparative example 7 | [C-7]                                 | (7)                             |
| Comparative example 8 | [C-8]                                 | (8)                             |

One of the two planographic printing plate precursors obtained for each of [C-1] to [C-8] was exposed by YAG laser emitting an infrared ray having a wavelength of 1064 nm at laser power: 360 mW and scanning speed: 2.0 m/s and the other of each of the plates was exposed by the YAG laser at laser power: 360 mW and scanning speed: 3.0 m/s. After the exposure, both plates were heated at 110° C. for 1 minute, then printed using a Hydel KOR-D Machine. In this procedure, it was observed whether blemishes occurred on non-image portions of the print or not. The results are shown in Table 6.

TABLE 6

|                       | Planographic printing plate precursor | Blemished on non-image portions in printing |                         |
|-----------------------|---------------------------------------|---------------------------------------------|-------------------------|
|                       |                                       | Scanning Speed: 2.0 m/s                     | Scanning Speed: 3.0 m/s |
| Comparative example 1 | [C-1]                                 | None                                        | slightly                |
| Comparative example 2 | [C-2]                                 | None                                        | slightly                |
| Comparative example 3 | [C-3]                                 | None                                        |                         |
| Comparative example 4 | [C-4]                                 | None                                        | slightly                |
| Comparative example 5 | [C-5]                                 | None                                        |                         |
| Comparative example 6 | [C-6]                                 | None                                        |                         |
| Comparative example 7 | [C-7]                                 | None                                        |                         |
| Comparative example 8 | [C-8]                                 | None                                        | slightly                |

As apparent from the results of Table 6, it was found that in the planographic printing plates of the comparative examples obtained by forming only a recording layer corresponding to layer (b) in the present invention, when exposed at a scanning speed of 2.0 m/s, there was no problem, however, when exposed at a scanning speed of 3.0 m/s, all of the resulting prints had blemishes on non-image portions, and there were problems with developability when exposed at low energy.

#### Examples of planographic printing plate (2) S-2

A coating solution having the composition described below was prepared using a sulfonic acid generating polymer (1p-7, GPC weight-average molecular weight: 20000, heat decomposition temperature by TGA: 155° C.). The resulting solution was coated on the hydrophilic treated surface of S-1 by a spin coater so that the amount coated after drying at 100° C. for 2 minutes was 0.3 g/m<sup>2</sup>. The substrate having the intermediate layer (layer (b)) thus

provided was called S-2. The surface had a contact angle against a water drop in air of 80°.

|    |                                       |      |
|----|---------------------------------------|------|
| 5  | (Intermediate layer coating solution) |      |
| 10 | Sulfonic acid generating polymer      | 5 g  |
|    | Methyl ethyl ketone                   | 80 g |
|    | Dimethylacetamide                     | 20 g |

## S-3

A substrate S-3 was obtained in the same manner as for S-2 except that a sulfonic acid generating polymer (1p-2, GPC weight-average molecular weight: 10000, heat decomposition temperature by TGA: 120° C.) was used and the amount coated was 0.2 g/m<sup>2</sup>. The surface had a contact angle against a water drop in air of 100°.

## S-4

A substrate S-4 was obtained in the same manner as for S-2 except that a sulfonic acid generating polymer (1p-8, GPC weight-average molecular weight: 50000, heat decomposition temperature by TGA: 134° C.) was used and the amount coated was 0.5 g/m<sup>2</sup>. The surface had a contact angle against a water drop in air of 90°.

## S-5

A substrate S-5 was obtained in the same manner as for S-2 except that a sulfonic acid generating polymer (1p-26, GPC weight-average molecular weight: 30000, heat decomposition temperature by TGA: 160° C.) was used and the amount coated was 1.0 g/m<sup>2</sup>. The surface had a contact angle against a water drop in air of 80°.

## S-6

A substrate S-6 was obtained in the same manner as for S-2 except that a sulfonic acid generating polymer (1p-25, GPC weight-average molecular weight: 30000, heat decomposition temperature by TGA: 155° C.) was used and the amount coated was 0.2 g/m<sup>2</sup>. The surface had a contact angle against a water drop in air of 80°.

## S-7

A substrate S-7 was obtained in the same manner as for S-2 except that a sulfonic acid generating polymer (1p-21, GPC weight-average molecular weight: 30000, heat decomposition temperature by TGA: 145° C.) was used and the amount coated was 0.2 g/m<sup>2</sup>. The surface had a contact angle against a water drop in air of 75°.

## S-8

A substrate S-8 was obtained in the same manner as for S-2 except that a carboxylic acid generating polymer (homopolymer having structure a-15, GPC weight-average molecular weight: 100,000) was used instead of the sulfonic acid generating polymer and the amount coated was 0.2 g/m<sup>2</sup>.

## S-9

A substrate S-9 was obtained by heating the substrate S-3 in an oven at 150° C. for 1 minute. Infrared absorption spectra of the surfaces of S-3 and S-9 were measured by the FT-IR diffusion reflection method. Absorptions at 1359 cm<sup>-1</sup> and 1099 cm<sup>-1</sup> derived from sulfonates observed in S-3 disappeared in S-9, and instead, absorptions at 1041 cm<sup>-1</sup> and 1012 cm<sup>-1</sup> derived from sulfonates were observed. Namely, it was found that the sulfonic acid generating ability of the sulfonic acid generating polymer contained in the intermediate layer coated on the substrate S-9 was lost. The

surface of the substrate S-9 had a contact angle against a water drop in air of 10° or less.

Examples 10 to 14, Comparative Examples 9, 10

Copper metal was deposited by vacuum deposition on the surfaces of the substrates S-2, S-3, S-4, S-7, S-8 and the hydrophilic substrate S-1 having the intermediate layer of the present invention obtained as described above, and the substrate S-9 having the intermediate layer containing no functional group represented by the general formulae (1) to (5) so as to form copper films having a thickness of 100 Å, to obtain the planographic printing plate precursors of Examples 10 to 14, and Comparative Examples 9 and 10, respectively. These were exposed image-wise by a YAG laser having an oscillation wavelength of 1064 nm, an output of 1 W, and a beam diameter of 20 mm, and offset printing was conducted using a Hydel KOR-D Machine. The resistance to blemishing of the resulting prints were evaluated visually according to the following standard.

Evaluation of blemish resistance

- No blemishing over a wide range of water/ink balance
- : Slight blemishing depending on water/ink balance

The results of the printing and the evaluation of blemish resistance are shown in the following Table 7.

Examples 15 to 19, Comparative Examples 11, 12

The printing plate precursors obtained in the above-described Examples 10 to 14, Comparative Examples 9 and 10 were stored for 3 days under conditions of a temperature of 60° C. and a humidity of 45% RH, then were exposed image-wise under the same conditions as in Example 1 and printing was conducted. The results are shown in Table 7 below.

TABLE 7

|                        | Polymer used in intermediate layer | Printing evaluation result                                                       |
|------------------------|------------------------------------|----------------------------------------------------------------------------------|
| Example 10             | 1 p-7 * <sup>1</sup>               | 10000 or more excellent prints were obtained. Blemishing resistance: ○           |
| Example 11             | 1 p-2 * <sup>1</sup>               | 10000 or more excellent prints were obtained. Blemishing resistance: ○           |
| Example 12             | 1 p-8 * <sup>1</sup>               | 10000 or more excellent prints were obtained. Blemishing resistance: ○           |
| Example 13             | 1 p-21 * <sup>1</sup>              | 10000 or more excellent prints were obtained. Blemishing resistance: ○           |
| Example 14             | a-15 * <sup>2</sup>                | 10000 or more excellent prints were obtained. Blemishing resistance: ○           |
| Comparative example 9  | No intermediate layer              | Whole surface was blemished significantly, and no image-wise print was obtained. |
| Comparative example 10 | Containing sulfonate group         | Image portions became faint after fewer than 100 prints.                         |
| Example 15             | 1 p-7 * <sup>1</sup>               | 10000 or more excellent prints were obtained.                                    |
| Example 16             | 1 p-2 * <sup>1</sup>               | About 5000 excellent prints were obtained.                                       |
| Example 17             | 1 p-8 * <sup>1</sup>               | 10000 or more excellent prints were obtained.                                    |
| Example 18             | 1 p-21 * <sup>1</sup>              | 10000 or more excellent prints were obtained.                                    |
| Example 19             | a-15 * <sup>2</sup>                | About 4000 excellent prints were obtained.                                       |
| Comparative example 11 | No intermediate layer              | Whole surface was blemished significantly, and no image-wise print was obtained. |

TABLE 7-continued

|                        | Polymer used in intermediate layer | Printing evaluation result                               |
|------------------------|------------------------------------|----------------------------------------------------------|
| Comparative example 12 | Sulfonate group * <sup>3</sup>     | Image portions became faint after fewer than 100 prints. |

\*<sup>1</sup>: Sulfonic acid generated polymer

\*<sup>2</sup>: Carboxylic acid generated polymer

\*<sup>3</sup>: 1 p-8 heated product, containing sulfonate group

When the planographic printing plates of the examples having the layer (b) and the layer (c) of the present invention were applied directly to a printing machine after exposure and printing was conducted, a large number of excellent prints were obtained, as is apparent from Table 7. Further, it was found from comparison between Example 10 and Example 14 that the print using a sulfonic acid generating polymer is more excellent than the print using a carboxylic acid generating polymer. This tendency did not change after storage of the planographic printing plate precursors at a high temperature and a high humidity, and it was found that the planographic printing plate precursors of the present invention have excellent storability at a high temperature and a high humidity.

30

Examples 20, 21, Comparative Examples 13

A coating solution having the composition described below was coated at a coating weight of 1 g/cm<sup>2</sup> as a recording layer (layer (c)) on the substrates S-5, S-6 and S-1 to obtain the planographic printing plate precursors of Examples 20 and 21 and Comparative Example 13, respectively. These plates were exposed using a YAG laser having an oscillation wavelength of 1064 nm, an output of 1 W and a beam diameter of 30 mm while the scanning speed was continuously changed. Printing was conducted using the resulting printing plates, and the line width at which it became impossible for ink to adhere by exposure was determined using a microscope, and exposing energy at the plate surface at which the line width was 30 mm was measured as a sensitivity value. The results are shown in Table 8 below.

35

55

Coating solution for recording layer

|                                                                                                |        |
|------------------------------------------------------------------------------------------------|--------|
| poly (α-methylstyrene)                                                                         | 1.0 g  |
| Infrared ray absorbing agent<br>(NK-3508, manufactured by Nippon Kanko Shikiso Kenkyusho K.K.) | 0.15 g |
| Dye in which counter ion in Victoria Pure Blue BOH is changed to 1-naphthalenesulfonic acid    | 0.05 g |
| Fluorine-based surfactant<br>(Megafack F-177, manufactured by Dainippon Ink & Chemicals, Inc.) | 0.06 g |
| Methyl ethyl ketone                                                                            | 20 g   |
| Methyl alcohol                                                                                 | 7 g    |

60

65

NK-3508



TABLE 8

|                        | Polymer used in intermediate layer | Sensitivity            |
|------------------------|------------------------------------|------------------------|
| Example 20             | 1 p-25 *1                          | 200 mJ/cm <sup>2</sup> |
| Example 21             | 1 p-21 *1                          | 200 mJ/cm <sup>2</sup> |
| Comparative example 13 | No intermediate layer              | 500 mJ/cm <sup>2</sup> |

\*1: Sulfonic acid generated polymer

As is apparent from Table 8, the planographic printing plates of the present invention have excellent sensitivity, and can provide excellent writing even by exposure at low energy.

#### Example 22

A planographic printing plate precursor was made in the same manner as in Example 20 except that the infrared ray absorbing agent in the recording layer was substituted by IR-125 (manufactured by Wako Pure Chemical Industries Ltd.). This plate precursor was exposed image-wise using a semiconductor laser having an oscillation wavelength of 840 nm and an output of 500 mW, then printing was conducted to obtain 10000 or more excellent prints having no faintness in image portions and no contamination on non-image portions at all.

#### Examples of planographic printing plate (3)

A thin film of Ti was made by vacuum deposition so that the thickness thereof was 300 Å as the layer (c), on the substrate S-1. The resulting sample was called M-1. Then, a coating solution having the composition described below was prepared. The resulting coating solution was coated on M-1 by a spin coater so that the amount coated after drying at 100° C. for 2 minutes was 1.0 g/m<sup>2</sup>. Thus, a printing plate precursor P-1 was obtained as Example 23. The surface of P-1 had a contact angle against a water drop in air of 80°.

|                                                                                                                                            |      |
|--------------------------------------------------------------------------------------------------------------------------------------------|------|
| Sulfonic acid generating polymer<br>(1p-7, GPC weight-average molecular weight: 20,000,<br>heat decomposition temperature by TGA: 155° C.) | 15 g |
| Methyl ethyl ketone                                                                                                                        | 80 g |
| Dimethylacetamide                                                                                                                          | 20 g |

The resulting P-1 was exposed image-wise with scanning using a semiconductor laser optical system having an oscillation wavelength of 840 nm, a beam diameter of 30 μm and an energy at the plate surface of 20 mW under conditions

15

where the energy concentration was 200 mJ/cm<sup>2</sup>. The obtained plate could be immediately subjected to offset printing using a Hydel KOR-D Machine to obtain 10000 or more excellent positive prints.

20

#### Comparative Example 14

Plate C-1 for comparison was obtained in the same manner as for the production of P-1 except that the layer (c) was not provided on the substrate S-1. The contact angle against a water drop in air of the surface of C-1 was 80°. Then, C-1 was heated in an oven at 150° C. for 1 minute, and the infrared absorption spectrum was measured before and after the heating. As a result, absorptions at 1359 cm<sup>-1</sup> and 1099 cm<sup>-1</sup> derived from sulfonates observed before the heating disappeared completely, and instead, absorptions at 1041 cm<sup>-1</sup> and 1012 cm<sup>-1</sup> derived from sulfonates were recognized. The surface after the heating had a contact angle against a water drop in air of 10° or less.

The substrate C-1 was used, and the whole surface was exposed with scanning using the same semiconductor laser optical system as in Example 23 under conditions where the energy concentration was 200 mJ/cm<sup>2</sup>. The contact angle against a water drop in air of the surface after exposure was 80°, and also regarding FT-IR, no change was recognized before and after the exposure. Further, scanning exposure was conducted image-wise using the same semiconductor laser optical system as in Example 1 under conditions where the energy concentration was 200 mJ/cm<sup>2</sup>, then immediately offset printing was conducted under the same conditions as for Example 23. As a result, ink adhered to the whole surface and no image was obtained at all.

50

#### Comparative Example 15

Further, M-1 on which the layer (b) was not provided in Example 23 was subjected to image-wise scanning exposure using the same semiconductor laser optical system as in Example 23 under conditions where the energy concentration was 200 mJ/cm<sup>2</sup>, then immediately offset printing was conducted under the same conditions as for Example 23. As a result, ink adhered to the whole surface and no image was obtained at all. When the exposure energy concentration was changed to 100 mJ/cm<sup>2</sup> and printing was conducted, prints were obtained, however, scratch-like adhesion was observed in image portions and printing durability of only 1000 sheets or less could be obtained.

The printing plate precursor P-1 in Example 23 has sufficient sensitivity for scanning exposure, and provides

55

60

65

excellent printing plates even without post treatment after exposure. Since the sulfonic acid generating polymer Ip-7 in layer (b) is excellent in heat sensitivity, as a result, P-1 has excellent discrimination of hydrophobicity/hydrophilicity before and after exposure. Further, P-1 has high sensitivity, and has excellent scratch resistance and printing durability as compared with the conventional printing plate precursor M-1 for heat mode exposure.

#### Examples 24 to 27

A printing plate precursor P-2 was produced as Example 24 in the same manner as in Example 23 except that the amount coated of a sulfonic acid generating polymer in layer (b) was changed to 2.0 g/m<sup>2</sup>. A printing plate precursor P-3 was produced as Example 25 in the same manner as in Example 23 except that the sulfonic acid generating polymer in the heat sensitive layer was changed to Ip-2 from Ip-7 and the amount coated was changed to 1.5 g/m<sup>2</sup>. A printing plate precursor P-4 was produced as Example 26 in the same manner as in Example 23 except that the sulfonic acid generating polymer in layer (b) was changed to Ip-8 from Ip-7 and the amount coated was changed to 1.2 g/m<sup>2</sup>. A printing plate precursor P-5 was produced as Example 27 in the same manner as in Example 23 except that the sulfonic acid generating polymer in layer (b) was changed to a-15 from Ip-7 and the amount coated was changed to 1.5 g/m<sup>2</sup>. The weight-average molecular weights and weight reduction temperatures in TGA of the polymers used in layer (b) are shown below.

Ip-7: GPC weight-average molecular weight: 50000

TGA weight reduction temperature: 155°C.

Ip-2: GPC weight-average molecular weight: 10000

TGA weight reduction temperature: 120°C.

Ip-8: GPC weight-average molecular weight: 25000

TGA weight reduction temperature: 134°C.

a-15: GPC weight-average molecular weight: 30000

10% by weight of cyclohexyl benzenesulfonate was added.

#### Comparative Examples 16 to 17

A printing plate precursor C-2 was produced as Comparative Example 16 in the same manner as in Comparative Example 14 except that the sulfonic acid generating polymer in layer (b) was changed to Ip-2 from Ip-7 and the amount coated was changed to 1.5 g/m<sup>2</sup>. A printing plate precursor C-3 was produced as Comparative Example 17 in the same manner as in Comparative Example 15 except that the intermediate layer of the Ti thin film having a thickness of 300 Å to a layer (c) of a Sn thin film having a thickness of 100 Å.

In Examples 24 to 27 and Comparative Examples 16 to 17, image-wise laser exposure was conducted in the same manner as in Example 23 and Comparative Examples 14 to 15, and printing was conducted using the prepared printing plates without further treatment. The printing durability, scratch resistance and blemishing resistance thereof were evaluated according to the following standards.

Printing durability: Faintness in the printed images was observed visually, and printing was continued until prints which could not be used in practice were obtained, and the printing number before that was counted.

Scratch resistance: Scratch-like ink adhesion on solid portions was observed visually, and evaluated according to the following standard.

○: No practical problem

✗: Unusable in practice

Blemishing resistance: The blemishing in non-image portions was observed visually while changing the water-ink balance in printing, and evaluated according to the following standard.

○: No blemishing over a very wide range of water-ink balance

○: No blemishing over a wide range of water-ink balance

Δ: Some blemishing depending on the water-ink balance

Evaluation results are shown in Table 9.

TABLE 9

| Structure of printing plate precursor |                  |                                 |                                 |                                                      |                     |                    |
|---------------------------------------|------------------|---------------------------------|---------------------------------|------------------------------------------------------|---------------------|--------------------|
| Form plate No.                        | (film thickness) | Intermediate layer component    | Heat sensitive layer polymer    | Exposure energy concentration                        | Printing result     |                    |
|                                       |                  |                                 |                                 |                                                      | Printing durability | Scratch resistance |
| P-2<br>(Example 24)                   | (150 Å)          | Ti                              | 1p-7<br>(2 g/m <sup>2</sup> )   | 175 mJ/cm <sup>2</sup>                               | 10000 or more       | ○ ○                |
| P-3<br>(Example 25)                   | (100 Å)          | Al                              | 1p-2<br>(1.5 g/m <sup>2</sup> ) | 250 mJ/cm <sup>2</sup>                               | 10000 or more       | ○ ○                |
| P-4<br>(Example 26)                   | (50 Å)           | Sn                              | 1p-8<br>(1.2 g/m <sup>2</sup> ) | 300 mJ/cm <sup>2</sup>                               | 10000 or more       | ○ ○                |
| P-5<br>(Example 27)                   | (700 Å)          | Ti                              | a-15<br>(1.5 g/m <sup>2</sup> ) | 300 mJ/cm <sup>2</sup>                               | 10000 or more       | ○ ○                |
| C-2<br>(Comparative example 16)       | None             | 1p-2<br>(1.5 g/m <sup>2</sup> ) | 1000 mJ/cm <sup>2</sup>         | Whole surface is blemished and no image is obtained. |                     |                    |
| C-3                                   | Sn               | None                            | 600 mJ/cm <sup>2</sup>          | 1000                                                 | ✗                   | Δ                  |

TABLE 9-continued

| Structure of printing plate precursor |                  | Heat sensitive layer polymer | Exposure | Printing result |                      |                     |
|---------------------------------------|------------------|------------------------------|----------|-----------------|----------------------|---------------------|
| Form plate No.                        | (film thickness) |                              |          | (amount coated) | energy concentration | Printing durability |
| (Comparative example 17)              | (100 Å)          |                              |          |                 |                      |                     |

## Example 28

A coating solution having the composition described below was coated as layer (c) on a substrate so that the weight coated was 0.3 g/m<sup>2</sup>, then, the same layer (b) as in Example 23 was provided. A plate precursor P-6 was obtained as Example 28. Then, P-6 was exposed image-wise with scanning using a YAG laser optical system having an oscillation wavelength of 1064 nm, a beam diameter of 20 μm and an energy at the plate surface of 500 mW under conditions where the energy concentration was 350 mJ/cm<sup>2</sup>. The obtained plate could be immediately subjected to offset printing to obtain 10000 or more sheets of excellent positive prints.

|                                                                   |       |
|-------------------------------------------------------------------|-------|
| Carbon black water dispersion (solid content: 34.4% by weight)    | 1.5 g |
| Polyvinylpyrrolidone (GPC weight-average molecular weight: 10000) | 1.5 g |
| Water                                                             | 100 g |
| Dimethylacetamide                                                 | 20 g  |

It was recognized that the printing plate precursors of Examples 24 to 28 having layers (b) and (c) have a high sensitivity to IR laser exposure, and provide a printing plate having excellent printability without post treatment after exposure, as is apparent from Table 9 and Example 28.

## Example 29

The above-described printing plate precursors P-1 to P-6 were produced and (A): some of them were exposed to a fluorescent light for 6 hours, (B): some of them were kept at a temperature of 45° C. and a humidity of 75% for 3 days, and (C) some of them were kept at a temperature of 60° C. and a humidity of 25%. All of them were exposed by laser, and printing evaluation was conducted. In the printing plate precursors exposed to conditions (A) to (C), no change was recognized in both drawing line width (sensitivity) and printability as compared with those directly after production and before exposure.

The planographic printing plate precursor of the present invention has sufficient scanning exposure sensitivity for practical use, and can provide a planographic printing plate having excellent printing durability, scratch resistance, and blemish resistance, without post treatment after exposure. Further, the planographic printing plate precursor of the present invention is a planographic printing plate precursor excellent in storage stability. The method for producing a

15 planographic printing plate of the present invention is simple and excellent in environmental aspects since it requires no post treatment, as compared with conventional production methods.

20 What is claimed is:

1. A planographic printing plate precursor obtained by laminating on a substrate (b) a layer composed of a hydrophobic polymer which can be made hydrophilic by heating, and (a) a layer composed of a hydrophilic polymer compound having in the side chain at least one of alkylene oxide groups or functional groups selected from —COOR, —COOM, —SOR, —SO<sub>2</sub>R, —SO<sub>3</sub>R, —SOM, —SO<sub>2</sub>M, —SO<sub>3</sub>M, —OH, and —NR<sup>22</sup>R<sup>23</sup> wherein, R represents a hydrogen atom, alkyl group, or aryl group, M represents a metal atom, R<sup>22</sup> and R<sup>23</sup> each independently represent a hydrogen atom, alkyl group, or aryl group and wherein the layer (a) and the layer (b) are laminated sequentially on the substrate.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 96

**69**

unsubstituted aryl group, R<sup>4</sup> represents a substituted or unsubstituted alkyl group, a substituted or unsubstituted aryl group, or —SO<sub>2</sub>—R<sup>5</sup>, R<sup>5</sup> represents a substituted or unsubstituted alkyl group or a substituted or unsubstituted aryl group, R<sup>6</sup> to R<sup>10</sup> each independently represent a hydrogen atom, or an alkyl group, alkenyl group, acyl group, or alkoxy carbonyl group which may have a substituent, R<sup>11</sup> represents an alkyl group or alkenyl group which may have a substituent, and any two of R<sup>6</sup> to R<sup>8</sup> or any two of R<sup>9</sup> to R<sup>11</sup> may be connected to form ring structure composed of 3 to 8 carbon atoms or hetero atoms.

3. A method for producing a planographic printing plate wherein the planographic printing plate precursor of claim 2

**70**

is exposed, and developed utilizing a developing solution mainly composed of water having a pH of 2 or more or wetting water on a printing machine.

4. A method for producing a planographic printing plate wherein the planographic printing plate precursor of claim 1 is subjected to heat mode exposure using an infrared laser light having a longer wavelength than 700 nm.

5. A planographic printing plate precursor according to claim 1, wherein the layer (a) further comprises a photo-thermal conversion material.

\* \* \* \* \*